# EUROPEAN PATENT SPECIFICATION

(11) **EP 1 321 301 B1**
(45) Date of publication and mention of the grant of the patent: **24.01.2007**
(21) Application number: 02080094.2
(22) Date of filing: 09.12.2002
(51) Int. Cl.: B41M 5/00

(54) **Multilayer ink recording element with porous organic particles**
Mehrschichtiges Tintenaufzeichnungselement mit organischen Partikeln
Matériau d'enregistrement d'encre multicouche et comprenant des particules organiques

(30) Priority: 20.12.2001 US 28129; 15.10.2002 US 271082
(43) Date of publication of application: 25.06.2003
(73) Proprietor: EASTMAN KODAK COMPANY, Rochester, New York 14650 (US)
(72) Inventor: Landry-Coltrain, C. J. T., Eastman Kodak Company, Rochester, New York 14650-2201 (US); Leon, Jeffrey W., Eastman Kodak Company, Rochester, New York 14650-2201 (US); Franklin, Linda M., Eastman Kodak Company, Rochester, New York 14650-2201 (US); Wang, Xiaoru, Eastman Kodak Company, Rochester, New York 14650-2201 (US)
(74) Representative: Haile, Helen Cynthia

(56) References cited:
- EP-A- 0 704 315
- EP-A- 0 825 296
- EP-A- 0 933 225
- EP-A- 1 318 025
- WO-A-02/07984
- US-A- 5 360 780
- DATABASE WPI Section Ch, Week 199014 Derwent Publications Ltd., London, GB; Class A97, AN 1990-103949 XP002260945 & JP 02 055186 A (CANON KK), 23 February 1990 (1990-02-23)

## Description

The invention relates to an ink recording element, more particularly to a multilayer ink recording element containing porous organic particles.

In a typical inkjet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water, an organic material such as a monohydric alcohol, a polyhydric alcohol or mixtures thereof.

An inkjet recording element typically comprises a support having on at least one surface thereof at least one ink-receiving or image-forming layer and includes those intended for reflection viewing, which have an opaque support, and those intended for viewing by transmitted light, which have a transparent support.

An inkjet recording element that simultaneously provides an almost instantaneous ink dry time and good image quality is desirable. However, given the wide range of ink compositions and ink volumes that a recording element needs to accommodate, these requirements of inkjet recording media are difficult to achieve simultaneously.

Inkjet recording elements are known that employ porous or non-porous single layer or multilayer coatings that act as suitable ink receiving layers on one or both sides of a porous or non-porous support. Recording elements that use non-porous coatings typically have good image quality and stability but exhibit poor ink dry time. Recording elements that use porous coatings typically contain colloidal particulates and have poorer image stability but exhibit superior dry times.

While a wide variety of different types of porous image recording elements for use with inkjet printing are known, there are many unsolved problems in the art and many deficiencies in the known products, which have severely limited their commercial usefulness. A major challenge in the design of a porous image-recording layer is to be able to obtain good quality, crack-free coatings. Inkjet prints, prepared by printing onto inkjet recording elements, are subject to environmental degradation. They are especially vulnerable to light fade and fade resulting from gaseous impurities in the air, such as ozone and nitrous oxide. Highly swellable hydrophilic layers can take an undesirably long time to dry, slowing printing speed. Porous layers speed the absorption of the ink vehicle, but often suffer from insufficient gloss and severe dye fade. Porous layers are also difficult to coat without cracking.

Japanese Kokai 07-137432 describes an inkjet paper having an ink-absorbing layer containing polyester resin particles with internal pores. However, there is a problem with this element in that the average particle size of the polyester resin is greater than 0.5 microns, and the element will have low surface gloss.

U.S. Pat No. 5,360,780 discloses an image-receiving sheet for thermal transfer printing comprising a substrate and an image-receiving layer disposed on said substrate, characterized in that said image-receiving layer contains thermoplastic resin fine particle aggregates, including polyester particles.

EP-A-0933225 discloses an image-transfer medium for ink-jet printing, comprising a base material, and a releasing layer and a transfer layer, both provided on the base material, wherein the transfer layer comprises fine particles of a thermoplastic resin, a thermoplastic resin binder, inorganic fine particles and a coupling agent.

EP-A-0825296 discloses matte finished coated paper and a process for manufacturing the same. The paper comprises a surface coating provided on at least one side of a web, which contains 3-14% by weight porous particles of an organic pigment each of which has a specified oil absorbency and 30-97% by weight calcium carbonate particles relative to the amount of pigment and each having a specified average particle diameter of 1.0 to 10 µm.

EP-A- 0704315 discloses an ink jet recording medium enabling the formation of a high quality image, and particularly an ink jet recording medium with a fabric substrate coated with porous particles having a particle size of from 0.1 to 30 µm, and a surface layer made of boehmite as the main component, formed on the substrate.

JP(A) 2055186 discloses a recording material used for ink jet recording comprising, in order, an ink holding layer and an ink penetration layer containing crosslinked soluble or hydrophilic polymer on a substrate. The ink penetration layer contains porous particles, which are, for example, polystyrene, polyester, polyvinyl ether, polyamide, urea resin, synthetic silica, clay talc or calcium carbonate. The recording element improves recording density, ink absorption and image contrast.

WO-A-0207984 discloses a recording medium for ink jet printing which may be employed for backlit or reflective light viewing. The printing medium includes a substrate, a first coating layer disposed on the substrate, and a second coating layer disposed on the second substrate, the second substrate having a microporous structure and comprising at least one hydrophobic polymer and at least one liquid absorbing filler dispersed substantially throughout the hydrophobic polymer.

EP-A-13108025 discloses an ink jet recording element including a support having thereon a fusible, porous, image-receiving layer having non-porous polymeric particles with a core/shell structure having a polymeric, hydrophobic core covered with a polymeric, hydrophobic shell, the Tg of the polymeric, hydrophobic core being at least 25° C higher than the Tg of the polymeric, hydrophobic shell.

It is an object of this invention to provide an ink recording element which will provide rapid ink uptake speed. Another objective of the invention is to provide an ink recording element having high surface gloss. Another objective of the invention is to provide an ink recording element having a receiving layer that when printed upon has an excellent image quality and stability.

The present invention comprises an ink recording element comprising a support and at least two ink receiving layers, wherein at least one of the at least two ink receiving layers comprises porous organic particles and is porous wherein said porous organic particles comprise unsaturated condensation polymer reacted with a vinyl monomer, and wherein said porous organic particles comprise at least 80 wt. % of an individual layer. In a preferred embodiment, at least one of the at least two ink receiving layers comprises porous polyester particles.

In one embodiment, at least one of the layers below the topmost layer may be porous and contain organic particles. In another embodiment, the porous layer containing organic particles may be the topmost layer of the ink recording element, in particular porous polyester particles having a mean diameter of less than 0.5 micrometers. Another embodiment may comprise a porous topmost layer containing organic particles and at least one lower porous layer containing organic particles. In a further embodiment, there may be multiple porous layers containing organic particles, which may also contain inorganic particles. In the most preferred embodiment, the porous organic particles comprise porous polyester particles.

The porous organic particles, which are preferably used in the invention may be in the form of porous beads, porous irregularly shaped particles, or may be aggregates of emulsion particles. Suitable porous organic particles, preferably polymeric, used in the invention comprise, for example, acrylic resins, styrenic resins, or cellulose derivatives, such as cellulose acetate, cellulose acetate butyrate, cellulose propionate, cellulose acetate propionate, and ethyl cellulose; polyvinyl resins such as polyvinyl chloride, copolymers of vinyl chloride and vinyl acetate and polyvinyl butyral, polyvinyl acetal, ethylene-vinyl acetate copolymers, ethylene-vinyl alcohol copolymers, and ethylene-allyl copolymers such as ethylene-allyl alcohol copolymers, ethylene-allyl acetone copolymers, ethylene-allyl benzene copolymers, ethylene-allyl ether copolymers, ethylene acrylic copolymers and polyoxy-methylene; polycondensation polymers, such as, polyesters or polyester-containing polymers, including polyethylene terephthalate, polybutylene terephthalate, polyurethanes and polycarbonates.

In a preferred embodiment of the invention, the porous organic particles, preferably polymeric, are made from a styrenic or an acrylic monomer. Any suitable ethylenically unsaturated monomer or mixture of monomers may be used in making such styrenic or acrylic polymer. There may be used, for example, styrenic compounds, such as styrene, vinyl toluene, p-chlorostyrene, vinylbenzylchloride or vinyl naphthalene; or acrylic compounds, such as methyl acrylate, ethyl acrylate, n-butyl acrylate, n-octyl acrylate, 2-chloroethyl acrylate, phenyl acrylate, methyl- α-chloroacrylate, methyl methacrylate, ethyl methacrylate, butyl methacrylate; and mixtures thereof. In another preferred embodiment, methyl methacrylate is used.

Typical crosslinking monomers used in making the porous organic particles, preferably polymeric, used in the invention may be aromatic divinyl compounds such as divinylbenzene, divinylnaphthalene or derivatives thereof; diethylene carboxylate esters and amides such as ethylene glycol dimethacrylate, diethylene glycol diacrylate, and other divinyl compounds such as divinyl sulfide or divinyl sulfone compounds. Divinylbenzene and ethylene glycol dimethacrylate are especially preferred. The porous polymeric particles have a degree of crosslinking of 27 mole % or greater, preferably 50 mole %, and most preferably 100 mole %. The degree of crosslinking is determined by the mole % of multifunctional crosslinking monomer which is incorporated into the porous organic particles, preferably polymeric.

The porous organic particles, used in this invention can be prepared, for example, by pulverizing and classification of porous organic compounds, by emulsion, suspension, and dispersion polymerization of organic monomers, by spray drying of a solution containing organic compounds, or by a polymer suspension technique which consists of dissolving an organic material in a water immiscible solvent, dispersing the solution as fine liquid droplets in aqueous solution, and removing the solvent by evaporation or other suitable techniques. The bulk, emulsion, dispersion, and suspension polymerization procedures are well known to those skilled in the polymer art and are taught in such textbooks as G. Odian in "Principles of Polymerization", 2nd Ed. Wiley (1981), and W.P. Sorenson and T.W. Campbell in "Preparation Method of Polymer Chemistry", 2nd Ed, Wiley (1968).

Techniques to synthesize porous organic polymer particles are taught, for example, in U.S. Patents 5,840,293; 5,993,805; 5,403,870; and 5,599,889, and Japanese Kokai Hei 5[1993]-222108. For example, an inert fluid or porogen may be mixed with the monomers used in making the porous polymer particles. After polymerization is complete, the resulting polymeric particles are, at this point, substantially porous because the polymer has formed around the porogen thereby forming the pore network. This technique is described more fully in U.S. Patent 5,840,293 referred to above.

A preferred method of preparing the porous organic particles, used in this invention includes forming a suspension or dispersion of ethylenically unsaturated monomer droplets containing the crosslinking monomer and a porogen in an aqueous medium, polymerizing the monomer to form solid, porous polymeric particles, and optionally removing the porogen by vacuum stripping. The particles thus prepared have a porosity as measured by a specific surface area of 35 m²/g or greater, preferably 100 m²/g or greater. The surface area is usually measured by B.E.T. nitrogen analysis known to those skilled in the art.

The porous organic particles may be covered with a layer of colloidal inorganic particles as described in U.S. Patents 5,288,598; 5,378,577; 5,563,226 and 5,750,378. The porous polymeric particles may also be covered with a layer of colloidal polymer latex particles as described in U.S. Patent 5,279,934.

The porous particles used in this invention have a median diameter of less than 10 µm, preferably less than 0.5 µm. Median diameter is defincd as the statistical average of the measured particle size distribution on a volume basis. For further details concerning median diameter measurement, see T. Allen, "Particle Size Measurement", 4th Ed., Chapman and Hall, (1990).

As noted above, the organic particles, preferably polymeric, used in the invention are porous. By porous is meant particles which either have voids or are permeable to liquids. These particles can have either a smooth or a rough surface.

The porous organic particles comprise an unsaturated condensation polymer reacted with a vinyl monomer. Porous, condensation polymer particles may be prepared by crosslinking an unsaturated precursor condensation polyester within an oil-in-water emulsion in the presence of a water-immiscible organic solvent. The crosslinked, porous condensation polymer particles may be prepared via methods which are analogous to those described below for porous polyester particles with the main difference being that an unsaturated precursor condensation polymer may be used in lieu of an unsaturated precursor polyester. The precursor condensation polymer may be a polymer containing a backbone consisting of repetitive organic diradicals linked together by one or more of the following bond types: amide, carbonate, urethane, ester, or urea bonds. Preferably, the precursor condensation polymer will contain ester bonds and one or more of non-ester bond types. In one embodiment, unsaturated condensation polymers comprises ester-co-urethane, ester-co-urea, ester-co-amide, ester-co-carbonate, most preferably ester-co-urethane or ester-co-carbonate. The polymer may be linear or branched.

The precursor condensation polymer will also contain chemical unsaturation through which it can be crosslinked within an oil-in-water emulsion in the presence of a water-immiscible organic liquid to afford porous particles. The chemical unsaturation may be present within the precursor polyester along the backbone, as functionalized end groups or as pendant groups. An example of the first case is a polyester-urethane of which one of the repetitive ester units is a maleate or fumarate moiety. An example of the second case is an alcohol-terminated polyurethane which has been reacted with methacryloyl chloride to afford methacrylate ester end groups. Preferably the chemical unsaturation will be present as backbone unsaturation.

The precursor condensation polymers may be synthesized using any of the techniques commonly known to those skilled in the art of polymer synthesis for preparing condensation polymers. In general, the methods involve the reaction of lewis acidic and lewis basic monomers, each with a functionalization number of two or more under solution or melt conditions. Specific reagent combinations are shown in Table 8. It should be noted that multifunctional reagents with functionality numbers other than 2 (for example, trifunctional, tetrafunctional) may also be used. Conditions may be chosen in which the different types of reagents will react in a single reactor. Alternately, a multiple stage approach may be used in which a prepolymer, macromonomer, or oligomer with appropriate terminating groups is reacted with one or more additional polyfunctional reagents in a subsequent step. For example, a polyester-carbonate may be prepared either by reacting a diacid chloride, a bischloroformate, and a diol in the same pot or by preparing a low molecular weight alcohol-terminated prepolymer, which is subsequently reacted with a bischloroformate.

**Table 8. Reagent combinations (difunctional cases) required for forming condensation polymers.**

| **Condensation polymer bond** | **Lewis acid** | **Lewis base** |
|---|---|---|
| Ester | Cyclic anhydride, diacid chloride, diester, diacid | Diol, diphenol |
| Urethane | Diisocyanate | Diol, diphenol |
| Urea | Diisocyanate, phosgene or derivative thereof | Diamine |
| Carbonate | Bischloroformate, phosgene or reactive derivative thereof | Diol, diphenol |
| Amide | Cyclic anhydride, diacid chloride, diester, diacid | Diamine |

The crosslinking reaction may be a radical-initiated polymerization of an ethylenically unsaturated monomer which readily copolymerizes with the unsaturated units in the precursor condensation polymer. The precursor condensation polymer can be organic-soluble, in which case an added emulsifying agent may be necessary. In another embodiment of this method, the precursor condensation polymer can be water-soluble, water-dispersible, or amphiphilic in character, in which case the precursor condensation polymer acts as the emulsifying species and an added emulsifying agent is merely optional. The methods by which the porous condensation polymer particles may be prepared as well as the other reagents used in the preparation (for example, emulsifiers, initiators, ethylenically unsaturated monomers, water-immiscible organic) are the same as those described below for the porous polyester particles. Preferably, the porous, condensation polymer particles will contain ionic groups, as described below for porous polyester particles. Preferably, these ionic groups will be quaternary ammonium moieties.

The porous, condensation polymer beads may have a mean diameter of 0.1 - 10 micron. Preferably, they will have a mean diameter of 0.1-0.5 micron.

The most preferred porous polyester particles useful for this invention consist of the free radical addition polymerization reaction product of an unsaturated precursor polyester with one or more vinyl monomers containing α,β ethylenic unsaturation. A precursor polyester is a polyester containing unsaturated groups which is used in turn to make porous polyester particles. The percent of total precursor polyester comprising the particles may be from 5-95% by weight. Preferably, the particles will contain 20-80% by weight of precursor polyester. The most preferred porous polyester particles may be crosslinked, and may be dispersible in water or water-miscible solvents. The porous structure may consist of either continuous or isolated pores.

The most preferred porous polyester particles of this invention may be prepared by any of several methods. These include the gradual, electrolyte-induced coalescence of smaller polyester particles, followed by swelling with a vinyl monomer and subsequent crosslinking, as described in Japanese Kokai 07/137432. Another method of preparation includes the polymerization of a water-in-oil-in-water emulsion in which the oil phase consists of a solution of an unsaturated polyester and one or more vinyl monomers as described in US patents 3,979,342 and 4,089,81.

A more preferred method of preparation is described in Serial Number 10/027,701 by Leon et al., (Docket 82842) "Method of Preparation of Porous Polyester Particles", in which the crosslinked, preferred porous polyester particles may be prepared by crosslinking an unsaturated precursor polyester within an oil-in-water emulsion in the presence of a water-immiscible organic solvent. The crosslinking reaction is a radical-initiated polymerization of an ethylenically unsaturated monomer, which readily copolymerizes with the unsaturated units in the precursor polyester. The precursor polyester can be organic-soluble, in which case an added emulsifying agent may be necessary. In another embodiment of this method, the precursor polyester can be water-soluble, water-dispersible, or amphiphilic in character, in which case the precursor polyester acts as the emulsifying species and an added emulsifying agent is merely optional. The water-immiscible organic solvent may be removed to yield a dispersion of porous, crosslinked, polyester-containing particles.

The precursor polyesters useful for the preparation of the preferred porous polyester particles of this invention may be branched or unbranched, contain chemical unsaturation, and may be soluble either in water-immiscible organic solvents or in water. Optionally, the precursor polyester may be self-emulsifying in water or amphiphilic or surfactant-like in character. The precursor polyesters may have any glass transition temperature, provided the precursor polyester fulfills the solubility requirements. Preferably, the number average molecular weight (Mn) is from 1,000 to 30,000 gm/mole.

As is well known in the art, polyesters are condensation products of polybasic acids or of corresponding acid equivalent derivatives such as esters, anhydrides or acid chlorides and polyhydric alcohols. It will be known that whenever "diacids" or "polyacids" are referred to in this document, that corresponding acid equivalent derivatives such as esters, anhydrides or acid chlorides are also included by reference. Polymerizable unsaturation may be introduced into the molecule by the selection of a polybasic acid or polyhydric alcohol, which contains α,β-ethylenic unsaturation. In most cases, the unsaturation will be contained within the polybasic acid unit. Optionally, one or more additional polyacids common in the art of polycondensation may be used in addition to the unsaturated polyacid. The ethylenically unsaturated polyacids include, but are not necessarily limited to maleic, fumaric, itaconic, phenylcnediacrylic, citraconic and mesaconic acid. Other, additional polyacids which do not contain chemical unsaturation and can be used in precursor polyesters are described in WO 01/00703. These diacids can include, but are not necessarily limited to malonic, succinic, glutaric, adipic, pimelic, azelaic, and sebacic acids, phthalic, isophthalic, terephthalic, tetrachlorophthalic, tetrahydrophthalic, trimellitic, trimesic, isomers of naphthalenedicarboxylic acid, chlorendic acid, trimellitic acid, trimesic acid, and pyromellitic acid.

Ethylenically unsaturated groups can also be introduced into the precursor polyester by synthetic modification. For example, a polyester with a high alcohol number can be reacted with an anhydride or acid chloride of acrylic acid or methacrylic acid in order to introduce ethylenically unsaturated units.

Precursor polyesters that may be suitable for the particles of this invention can furthermore be comprised of any of a wide variety of polyhydric alcohols which are well known in the art of polycondensation and may be aliphatic, alicyclic, or aralkyl. A description of suitable polyhydric alcohols is given in WO 01/00703. These alcohols can include, but are not necessarily limited to ethylene glycol, 1,3-propylene glycol, 1,6-hexanediol, 1,10-decanediol, 1,4-cyclohexanedimethanol, 1,4-cyclohexanediol, hydroquinone bis (hydroxyethyl) ether, diethylene glycol, neopentyl glycol, bisphenols such as bisphenol A, ethylene oxide and propylene oxide adducts of bisphenol A, pentaerythritol, trimethylolpropane, and polyester polyols, such as that obtained by the ring-opening polymerization of ε-caprolactone. Additionally, A-B type polycondensation monomers which contain both hydroxyl and acid derivative functions can be used as well as monoacids and monoalcohols.

In one variation of this method of preparation, precursor polyesters which may be water-soluble, surfactant-like, or self-emulsifying and additionally contain chemical unsaturation may be utilized. Water-soluble, surfactant-like, and self-emulsifying precursor polyesters are well known in the art and will contain one or more types of hydrophilic chemical group or functionality, or monomer, such as carboxylate, quaternary ammonium, sulfonate, sulfate, sulfonium, phosphonium, iminosulfonyl, or polymeric or oligomeric oxyethylene segments. Precursor polyesters used to form the preferred porous polyester particles useful in this invention will additionally contain one or more polyacid or polyol monomers which contain ethylenic unsaturation as detailed above. The water-soluble, surfactant-like, and self-emulsifying precursor polyesters used to form the preferred porous polyester particles useful in this invention may contain one or more diacid or diol components which can induce hydrophilic character or water-solubility. The most common hydrophilic diol used for this purpose is polyethylene glycol. Additionally, tertiary amine units substituted with two or three hydroxyalkyl groups can be incorporated within a precursor polyester and rendered ionic either by quaternization with an alkylating agent or by neutralization with an acid. A commonly used class of diacid components used to impart hydrophilicity to precursor polyesters includes compounds containing sulfonate or sulfonimide salts. Some suitable sulfonated diacids are described in U.S. patents 4,973,656 and 5,218,042. Examples of such diacids are 5-sodiosulfoisophthalic acid, 2-sodiosulfobutanoic acid, and di-Me sodioiminobis(sulfonyl-*m*-benzoate). Another common strategy for the hydrophilization of precursor polyesters involves the neutralization of the acid end groups of polyester with a relatively high acid number. Preferably, the acid number is at least 10. Most preferably the acid number is greater than 25. The neutralization agent may be usually an alkali metal hydroxide or an amine. Precursor polyesters containing ethylenic unsaturation and neutralized acid end groups can also be used in this invention. In the preferred case, the unsaturated precursor polyester will contain an ionic group equivalent weight of from 400 to 2000 grams of polymer per mole of ionic unit.

The ethylenically unsaturated monomers useful for crosslinking the precursor polyesters in the particles of this invention may be monomers commonly used in the art of addition polymerization. These include, but are not necessarily limited to methacrylic acid esters, such as methyl methacrylate, ethyl methacrylate, isobutyl methacrylate, 2-ethylhexyl methacrylate, benzyl methacrylate, phenoxyethyl methacrylate, cyclohexyl methacrylate and glycidyl methacrylate, acrylate esters such as methyl acrylate, ethyl acrylate, isobutyl acrylate, 2-ethylhexyl acrylate, benzyl methacrylate, phenoxyethyl acrylate, cyclohexyl acrylate, and glycidyl acrylate, styrenics such as styrene, α-methylstyrene, 3- and 4-chloromethylstyrene, halogen-substituted styrenes, and alkyl-substituted styrenes, vinyl halides and vinylidene halides, N-alkylated acrylamides and methacrylamides, vinyl esters such as vinyl acetate and vinyl benzoate, vinyl ethers, such as butyl vinyl ether and cycloxexanedimethanol divinyl ether, allyl alcohol and its ethers and esters, and unsaturated ketones and aldehydes such as acrolein and methyl vinyl ketone and acrylonitrile.

In addition, small amounts (typically less than 10% of the total weight of the polymerizeable solids) of one or more water-soluble ethylenically unsaturated monomer can be used. Such monomers include but are not necessarily limited to styrenics, acrylates, and methacrylates substituted with highly polar groups, unsaturated carbon and heteroatom acids such as acrylic acid, methacrylic acid, fumaric acid, maleic acid, itaconic acid, vinylsulfonic acid, vinylphosphonic acid, and their salts, vinylcarbazole, vinylimidazole, vinylpyrrolidone, and vinylpyridines.

Especially useful in the polyester particles of this invention are monomers containing more than one ethylenically unsaturated unit, such as trimethylolpropane triacrylate, ethylene glycol dimethacrylate, isomers of divinylbenzene, divinyl adipate, cyclohexanedimethanol divinyl ether and ethylene glycol divinyl ether.

Ethylenically unsaturated monomers which may be preferred for the particles of this invention are styrenics, vinyl ethers, and methacrylates. Divinylbenzene (m, and p isomers), styrene, divinyl adipate, and ethylene glycol dimethacrylate are especially preferred.

Any of the common water-soluble or organic-soluble free radical polymerization initiators known in the art of addition polymerization can be used for the particles of this invention. These include, but are not restricted to azo compounds, such as 2,2'-azobis(4-methoxy-2,4-dimethylvaleronitrile), (1-pheneylethyl)azodiphenylmethane, 2-2'-azoisobutyronitrile (AIBN), 1,1'-azobis(1-cyclohexanedicarbonitrile), 4,4'-azobis(4-cyanopentanoic acid), and 2,2'-azobis(2-amidinopropane) dihydrochloride, organic peroxides, organic hydroperoxides, pcresters, and peracids such as benzoyl peroxide, lauryl peroxide, capryl peroxide, acetyl peroxide, t-butyl hydroperoxide, t-butyl perbenzoate, cumyl hydroperoxide, peracetic acid, 2,5-dimethyl-2,5-di(peroxybenzoate), and p-chlorobenzoly peroxide, persulfate salts such as potassium, sodium and ammonium persulfate, disulfides, tetrazenes, and redox initiator systems such as H₂O₂/Fe²⁺, persulfate/bisulfite, oxalic acid/Mn³⁺, thiourea/Fe³⁺, and benzoyl perozide/dimethylaniline.

Optionally, a small amount of a cosurfactant stabilizer, typically comprising 1-10% by weight of the organic phase, may be added to the organic phase. These hydrophobic compounds are known to prevent Ostwald ripening in certain types of emulsion and suspension polymerization. Excellent discussions of cosurfactants are given in *Emulsion Polymerization and Emulsion Polymers* by Peter A Lovell and Mohammed S. El-Aaser, (John Wiley and Sons: Chichester, 1997, pp. 700-721) and US Patent 5,858,634. The most common cosurfactants are hexadecane and hexadecanol. Other useful cosurfactants may also serve other roles, such as acting as monomers or initiators. An example of the former is lauryl methacrylate. An example of the latter is lauroyl peroxide.

If a precursor polyester is used, which is not soluble or dispersible in water, then an emulsifier may be additionally be used, although an emulsifier can be used in tandem with a water-soluble or water-dispersible precursor polyester. It may be preferable that the emulsifier be initially dissolved in the aqueous phase. Though a very large variety of emulsifiers are known in the art, most of these fit into the three basic categories of surfactants, colloidal inorganics, and protective colloids. There exist a tremendous number of known surfactants. Good reference sources for surfactants are the *Surfactant Handbook* ( GPO: Washington, D. C., 1971) and *McCutcheon's Emulsifiers and Detergents* (Manufacturing Confectioner Publishing Company: Glen Rock, 1992). There are no general restrictions for the surfactants which may be useful in the preparation of porous polyester particles. Useful surfactants can be anionic, cationic, zwitterionic, neutral, low molecular weight, macromolecular, synthetic, or extracted or derived from natural sources. Some examples include, but are not necessarily limited to: sodium dodecylsulfate, sodium dodecylbenzenesulfonate, sulfosuccinate esters, such as those sold under the AEROSOL^{®} trade name, flourosurfactants, such as those sold under the ZONYL^{®} and FLUORAD^{®} trade names, ethoxylated alkylphenols, such as TRITON^{®} X-100 and TRITON^{®} X-705, ethoxylated alkylphenol sulfates, such as RHODAPEX^{®} CO-436, phosphate ester surfactants such as GAFAC^{®} RE-90, hexadecyltrimethylammonium bromide, polyoxyethylenated long-chain amines and their quaternized derivatives, ethoxylated silicones, alkanolamine condensates, polyethylene oxide-copolypropylene oxide block copolymers, such as those sold under the PLURONIC^{®} and TECTRONIC^{®} trade names, N-alkylbetaines, N-alkyl amine oxides, and fluorocarbon-poly(ethylene oxide) block surfactants, such as FLUORAD^{®} FC-430.

Protective colloids useful in the preparation of porous polyester particles include, but are not necessarily limited to: poly (ethylene oxide), hydroxyethyl cellulose, poly (vinyl alcohol), poly (vinyl pyrrolidone), polyacrylamides, polymethacrylamides, sulfonated polystyrenes, alginates, carboxy methyl cellulose, polymers and copolymers of dimethylaminoethylmethacrylate, water soluble complex resinous amine condensation products of ethylene oxide, urea and formaldehyde, polyethyleneimine, casein, gelatin, albumin, gluten and xanthan gum. Protective colloids are a class of emulsifiers which may be used in lieu of or in addition to a surfactant. They may be typically dissolved or dispersed in the aqueous phase prior to the emulsification step.

Similarly, colloidal inorganic particles can be employed as emulsifiers as part of a limited coalescence process. Colloidal inorganic particles can be employed in lieu of or in addition to any other type of emulsifier listed, such as a surfactant or protective colloid. They may be also dispersed in the aqueous phase. Limited coalescence techniques have been describe in numerous patents such as U.S. Patents 4,833,060 and 4,965,131. A colloidal inorganic which is particularly useful in this invention is LUDOX^{®} TM sold by Du Pont.

Additional additives which can be incorporated into the preferred porous polyester particles useful in this invention include pigments, dyes, biocides, fungicides, electrolytes, buffers, UV-absorbers, antioxidants and chain transfer agents.

The preferred porous polyester particles useful for this invention comprise porous polyester particles having a mean diameter of from less than 0.1 micrometers to 10 micrometers. When the porous polyester particles are in the topmost layer, it is preferable that the porous polyester particles have a mean diameter range from 0.1 to less than 0.5 micrometers, and more preferably, that the porous polyester particles have a mean diameter range from 0.2 to 0.3 micrometers. An ink recording element having porous polyester particles with a mean diameter less than 0.5 micrometers preferably provides a surface gloss of greater than or equal to 10 at a measurement angle of 60 degrees. For optimal ink absorption properties and coating quality of the lower layer(s), it is preferable that the porous polyester particles have a mean diameter greater than 0.5 micrometers, preferably having a mean diameter from 1 to 10 micrometers, and most preferably having a mean diameter from 1 to 3 micrometers. The diameter of the particles can be measured by any method known in the art. One such method may be laser light scattering of dilute dispersions of the particles, using a commercially available instrument such as the Horiba LA-920, manufactured by Horiba LTD. Typically, a sample of preferred porous polyester particles will contain a population of particles having a distribution of sizes. This is the particle size distribution, and is characterized by a mean diameter, a standard deviation, and a coefficient of variation. The mathematical equations defining these terms can be found in any basic text on statistical analysis, such as "Principles of Instrumental Analysis, 4^{th} Edition", by D. A. Skoog and J. J. Leary, Harcourt Brace College Publishers, Orlando, FL, 1971 (Appendix A-6). The mean diameter is the arithmetic mean of the particle size distribution. The coefficient of variation (CV) of a distribution is the ratio of the standard deviation of the distribution to the mean diameter, given as a percent. The preferred porous polyester particles useful for this invention can have a relatively large distribution of particle sizes within one mode. In a system of particles, there can be a single mode or peak to this distribution of sizes, or there can be several modes, each mode being characterized by a mean diameter, a standard deviation, and a coefficient of variation. For example, the porous polyester particles can be a system composed of particles having a mode with a mean diameter of less than 0.5 micrometers and particles having a mode with mean diameter greater than 0.5 micrometers, preferably having a mean diameter from 1 to 10 micrometers, and most preferably having a mean diameter from 1 to 3 micrometers. The relative proportions of these two modes are calculated from the relative areas under the curves representing the modes, and should add up to 100 %.

In the preferred case, the porous polyester particles will contain an ionic group equivalent weight of from 40 to 2000 grams per mole of ionic unit. In one embodiment, the ionic group may preferably comprise sulfonate functionality. The product particles, having excellent colloidal stability, can be stored as an aqueous dispersion or freeze dried to yield a solid powder comprising dry particles which will easily redisperse in water.

The ink receiving element utilized in the invention contains at least two individual ink receiving layers. Each layer being comprised of a different composition, combination of particles with differing chemical nature and different mean diameters, and layer thickness. For these multilayer structures, the terms as used herein, "top", "upper", and "above" mean the layer that is farther from the support in relation to the relative positioning with respect to the other layers. The terms "bottom" "lower" and "below" mean the layer that is closer to the support in relation to the relative positioning with respect to the other layers. The term "topmost" means the layer that is the farthest from the support relative to all other layers.

The element of the present invention may contain other, including non-porous particles, as well. These particles may be organic or inorganic. The organic particles in any of the layers useful for this invention include non-coalescing latex particles and core-shell latex particles, such as polyolefins, polyethylene, polypropylene, polystyrene, poly(styrene-co-butadiene), polyurethane, polyester, poly(acrylate), poly(methacrylate), copolymers of n-butylacrylate and ethylacrylate, copolymers of vinylacetate and n-butylacrylate, copolymers of methyl methacrylate and sodium 2-sulfo-1,1-dimethylethyl acrylamide, and copolymers of ethyl acrylate, vinylidene chloride and sodium 2-sulfo-1,1-dimethylethyl acrylamide or mixtures thereof. These can be internally crosslinked or uncrosslinked. It may be preferable that uncrosslinked latex particles have a film formation temperature above 25 °C. Organic particles useful for this invention can also be porous acrylic, methacrylic, or styrenic polymer particles.

More specifically, organic particles which may be used in the invention include polymeric particles such as, for example, particles made from acrylic resins, styrenic resins, or cellulose derivatives, such as cellulose acetate, cellulose acetate butyrate, cellulose propionate, cellulose acetate propionate, and ethyl cellulose; polyvinyl resins such as polyvinyl chloride, copolymers of vinyl chloride and vinyl acetate and polyvinyl butyral, polyvinyl acetal, ethylene-vinyl acetate copolymers, ethylene-vinyl alcohol copolymers, and ethylene-allyl copolymers such as ethylene-allyl alcohol copolymers, ethylene-allyl acetone copolymers, ethylene-allyl benzene copolymers, ethylene-allyl ether copolymers, ethylene acrylic copolymers and polyoxy-methylene; polycondensation polymers, such as, polyesters or polyester-containing polymers, including polyethylene terephthalate, polybutylene terephthalate, polyurethanes and polycarbonates. Examples of organic particles useful in the invention are disclosed and claimed in U.S. Patent Application Serial Numbers: 09/458,401, filed Dec. 10, 1999; 09/608,969, filed June 30, 2000; 09/607,417, filed June 30, 2000; 09/608,466 filed June 30, 2000; 09/607,419, filed June 30, 2000; and 09/822,731, filed March 30, 2001.

The inorganic particles in any of the layers useful for this invention include any inorganic oxide, including silica, colloidal silica, fumed silica, alumina, colloidal alumina, fumed alumina, calcium carbonate, kaolin, talc, calcium sulfate, natural or synthetic clay, barium sulfate, titanium dioxide, silicon dioxide, zinc oxide, or mixtures thereof. Mixtures of organic and inorganic particles may also be used.

The organic particles and inorganic particles can be of any size, however, it is preferable that their mean particle diameter be of less than 0.5 micrometers if the layer containing these particles is the topmost layer. Organic and inorganic particles may also be present in the same or separate layers.

The polymers useful in any of the layers free of particles for this invention, including the topmost layer, include hydrophilic organic polymers and lightly crosslinked hydrogels such as polyvinylpyrrolidone and vinylpyrrolidone-containing copolymers, polyethyloxazoline and oxazoline-containing copolymers, imidazole-containing polymers, polyacrylamides and acrylamide-containing copolymers, poly(vinyl alcohol) and vinyl-alcohol-containing copolymers, poly(vinyl methyl ether), poly(vinyl ethyl ether), poly(alkylene oxide), gelatin, cellulose ethers, poly(vinylacetamides), partially hydrolyzed poly(vinyl acetate/vinyl alcohol), poly(acrylic acid), sulfonated or phosphated polyesters and polystyrenes, casein, albumin, chitin, chitosan, dextran, pectin, collagen derivatives, collodian, agar-agar, arrowroot, guar, carrageenan, tragacanth, xanthan, rhamsan, hydroxyethyl cellulose, hydroxypropyl cellulose, hydroxypropyl methyl cellulose, methyl cellulose, a poly(alkylene oxide), and water dispersible polyurethane. Mixtures of the above listed hydrophilic polymers can be used.

The ink receiving layers of the inkjet element may be formed by coating a mixture comprised of either the preferred porous polyester particles, organic particles, or inorganic particles and a binder in an amount insufficient to alter the porosity of the porous receiving layers onto a support, and then drying to remove approximately all of the volatile components. The binder preferably comprises an organic binder. In a preferred embodiment, the polymeric binder is a hydrophilic polymer such as polyvinylpyrrolidone and vinylpyrrolidone-containing copolymers, polyethyloxazoline and oxazoline-containing copolymers, imidazole-containing polymers, polyacrylamides and acrylamide-containing copolymers, poly(vinyl alcohol) and vinyl-alcohol-containing copolymers, poly(vinyl methyl ether), poly(vinyl ethyl ether), poly(alkylene oxides), gelatin, cellulose ethers, poly(vinylacetamides), partially hydrolyzed poly(vinyl acetate/vinyl alcohol), poly(acrylic acid), sulfonated or phosphated polyesters and polystyrenes, casein, albumin, chitin, chitosan, dextran, pectin, collagen derivatives, collodian, agar-agar, arrowroot, guar, carrageenan, tragacanth, xanthan, rhamsan. In another preferred embodiment of the invention, the hydrophilic polymer is hydroxyethyl cellulose, hydroxypropyl cellulose, hydroxypropyl methyl cellulose, methyl cellulose, or a poly(alkylene oxide). In still another preferred embodiment, the polymeric binder is a latex such as poly(styrene-co-butadiene), polyurethane, polyester, poly(acrylate), poly(methacrylate), a copolymer of n-butylacrylate and ethylacrylate, and a copolymer of vinylacetate and n-butylacrylate. In still another preferred embodiment, the binder may be a condensate of alkoxysilanes or other metal sols such as alumina sol, titania sol, or zirconia sol. Mixtures of the above listed hydrophilic polymers can be used. The binder should be chosen so that it is compatible with the aforementioned particles.

The amount of polymer binder used should be sufficient to impart cohesive strength to the ink recording element, such as an inkjet recording element, but should also be minimized so that the interconnected pore structure formed by the aggregates is not filled in by the binder. In a preferred embodiment of the invention, the polymer binder is present in an amount of from 5 to 50 % by weight, and most preferably, in an amount from 10 to 25 % by weight of each layer. The porous polymer particles comprise from 50 to 95% by weight of an individual layer. The particles preferably comprise from 75 to 90% by weight of an individual layer and most preferably comprise at least 80 wt. % of an individual layer.

The total thickness of the combined ink receiving layers may range from 5 to 100 µm, preferably from 10 to 50 µm. Each layer may have a different thickness relative to the other layers. However, it is typical that the topmost layer be thin relative to the lower layers. A preferred thickness of the topmost layer is from 1 to 20 µm, more preferably from 1 to 10 µm. The coating thickness required is determined through the need for the coating to act as a sump for absorption of ink solvent and the need to hold the ink near the coating surface.

Since the image recording element may come in contact with other image recording articles or the drive or transport mechanisms of image recording devices, additives such as filler particles, surfactants, lubricants, crosslinking agents, matte particles may be added to the element to the extent that they do not degrade the properties of interest.

Filler particles may be used in the ink receiving layer containing preferred porous polyester particles such as silicon oxide, fumed silica, silicon oxide dispersions such as those available from Nissan Chemical Industries and DuPont Corp., aluminum oxide, fumed alumina, calcium carbonate, barium sulfate, barium sulfate mixtures with zinc sulfide, inorganic powders such as γ-aluminum oxide, chromium oxide, iron oxide, tin oxide, doped tin oxide, alumino-silicate, titanium dioxide, silicon carbide, titanium carbide, and diamond in fine powder, as described in U.S. Patent 5,432,050.

A dispersing agent, or wetting agent can be present to facilitate the dispersion of the filler particles. This helps to minimize the agglomeration of the particles. Useful dispersing agents include, but are not limited to, fatty acid amines and commercially available wetting agents such as Solsperse® sold by Zeneca, Inc. (ICI). Preferred filler particles are silicon oxide, aluminum oxide, calcium carbonate, and barium sulfate. Preferably, these filler particles have a median diameter less than 1.0 µm. The filler particles can be present in the amount from 0 to 80 percent of the total solids in the dried ink receiving layer, most preferably in the amount from 0 to 40 percent.

In order to obtain adequate coatability, rheology modifiers known to those familiar with such art such as thickening agents or polymers may be used. These include associative thickeners such as hydrophobically modified hydroxyethylcellulose, hydrophobically modified alkali-soluble or alkali swellable emulsions, and hydrophobically modified ethylene oxide urethane block copolymers such as those supplied by Rohm & Haas under the trade name of Acusol ® and Dow Chemical under the trade name of Polyphobe®, and non-associative thickeners such as hydroxyethyl cellulose, hydroxypropyl methyl cellulose, sodium carboxy methyl cellulose, xanthan gum, guargum, and carrageenan.

The inkjet element may include lubricating agents. Lubricants and waxes useful either in the ink receiving layers or on the side of the element that is opposite the ink receiving layers include, but are not limited to, polyethylenes, silicone waxes, natural waxes such as carnauba, polytetrafluoroethylene, fluorinated ethylene propylene, silicone oils such as polydimethylsiloxane, fluorinated silicones, functionalized silicones, stearates, polyvinylstearate, fatty acid salts, and perfluoroethers. Aqueous or non-aqueous dispersions of submicron size wax particles such as those offered commercially as, but not limited to, dispersions of polyolefins, polypropylene, polyethylene, high density polyethylene, microcrystalline wax, paraffin, natural waxes such as carnauba wax, and synthetic waxes from such companies as Chemical Corporation of America (Chemcor), Inc., Michelman Inc., Shamrock Technologies Inc., and Daniel Products Company, may be useful.

In order to obtain adequate coatability, additives known to those familiar with such art such as surfactants, defoamers, alcohol may be used. Coating aids and surfactants include, but are not limited to, nonionic fluorinated alkyl esters such as FC-430®, FC-431®, FC-10®, FC-171® sold by Minnesota Mining and Manufacturing Co., Zonyl® fluorochemicals such as Zonyl-FSN®, Zonyl-FTS®, Zonyl-TBS®, Zonyl-BA® sold by DuPont Corp., other fluorinated polymer or copolymers such as Modiper F600® sold by NOF Corporation, polysiloxanes such as Dow Coming DC 1248®, DC200®, DC510®, DC 190® and BYK 320®, BYK 322®, sold by BYK Chemie and SF 1079®, SF1023®, SF 1054®, and SF 1080® sold by General Electric, and the Silwet® polymers sold by Union Carbide, polyoxyethylene-lauryl ether surfactants, sorbitan laurate, palmitate and stearates such as Span® surfactants sold by Aldrich, poly(oxyethylene-co-oxypropylene) surfactants such as the Pluronic® family sold by BASF, and other polyoxyethylene-containing surfactants such as the Triton X® family sold by Union Carbide, ionic surfactants, such as the Alkanol® series sold by DuPont Corp., and the Dowfax® family sold by Dow Chemical. Specific examples are described in MCCUTCHEON's Volume 1: Emulsifiers and Detergents, 1995, North American Edition.

The ink receiving layers may include crosslinking agents. Any crosslinking agent may be used provided its reactive functionalities have the appropriate reactivity with specific chemical units in the binder. Some common crosslinkers which can crosslink binders rich in lewis basic functionalities include, but are not necessarily limited to: carbodiimides, polyvalent metal cations, organic isocyanates such as tetramethylene diisocyanate, hexamethylene diisocyanate, diisocyanato dimethylcyclohexane, dicyclohexylmethane diisocyanate, isophorone diisocyanate, dimethylbenzene diisocyanate, methylcyclohexylene diisocyanate, lysine diisocyanate, tolylene diisocyanate, diphenylmethane diisocyanate, aziridines such as taught in U. S. Patent 4,225,665, ethyleneimines such as Xama-7® sold by EIT Industries, blocked isocyanates such as CA BI-12 sold by Cytec Industries, melamines such as methoxymethylmelamine as taught in U. S. Patent 5,198,499, alkoxysilane coupling agents including those with epoxy, amine, hydroxyl, isocyanate, or vinyl functionality, Cymel® crosslinking agents such as Cymel 300®, Cymel 303®, Cymel 1170®, Cymel 1171® sold by Cytec Industries, and bis-epoxides such as the Epon® family sold by Shell. Other crosslinking agents include compounds such as aryloylureas, aldehydes, dialdehydes and blocked dialdehydes, chlorotriazines, carbamoyl pyridiniums, pyridinium ethers, formamidinium ethers, vinyl sulfones, boric acid, dihydroxydioxane, and polyfunctional aziridines such as CX-100 (manufactured by Zeneca Resins). Such crosslinking agents can be low molecular weight compounds or polymers, as discussed in U. S. Patent 4,161,407 and references cited.

To improve colorant fade, UV absorbers, radical quenchers or antioxidants may also be added to the ink-receiving layers as is well known in the art. Examples include polyalkylenepolyamine-dicyanodiamide based polycondensation products, water soluble reducing agents, such as sulfites, nitrites, phosphates, thiosulfates, ascorbic acid or salts thereof, hydroxylamine derivatives, and glucose, sulfur-containing compounds, such as thiocyanates, thiourea, 2-mercaptobenzimidazole, 2-mercaptobenzthiazole, 2-mercaptobenzoxazole, 5-mercapto-1-methyl-tetrazole, 2,5-dimercapto-1,3,4-triazole, 2,4,6-trimcrcaptocyanuric acid, thiosalicylic acid, thiouracil, 1,2-bis(2-hydroxycthylthio)ethane, or hydrophobic antioxidant emulsified dispersions, such as hindered phenol based antioxidants, piperidine based antioxidants or hindered amines. UV absorbers include those described in Japanese Patent Publication Open to Public Inspection Nos. 57-74193, 57-87988, and 2-261476, antifading agents include those described in Japanese Patent Publication Open to Public Inspection Nos. 57-74192, 57-87989, 60-72785, 61-146591, 1-95091, and 3-13376.

The ink receiving layers may include pH modifiers, adhesion promoters, rheology modifiers, latexes, biocides, dyes, optical brighteners, whitening agents, described in Japanese Patent Publication Open to Public Inspection Nos. 59-42993, 59-52689, 62-280069, 61-242871, and 4-219266, and antistatic agents.

The ink receiving layers utilized in the invention can contain one or more mordanting species or polymers. The mordant polymer can be a soluble polymer, a charged molecule, or a crosslinked dispersed microparticle. The mordant can be non-ionic, cationic or anionic. Examples of a mordant are polymers or copolymers containing a quaternized nitrogen moiety, such as, for example, poly(styrene-co-1-vinylimidazole-co-1-vinyl-3-benzylimidazolium chloride), poly(styrene-co-1-vinylimidazole-co-1-vinyl-3-hydroxyethyl-imidazolium chloride), poly(styrene-co-1-vinylimidazole-co-1-vinyl-3-benzylimidazolium chloride-co-1-vinyl-3-hydroxyethylimidazolium chloride), poly(vinylbenzyltrimethylammonium chloride-co-divinylbenzene), poly(ethyl acrylate-co-1-vinylimidazole-co-1-vinyl-3-benzylimidazolium chloride), or poly(styrene-co-4-vinylpyridine-co-4-hydroxyethyl-1-vinylpyridinium chloride). In a preferred embodiment of the invention, the quaternary nitrogen moiety incorporated in the polymer is a salt of trimethylvinylbenzylammonium, benzyldimethylvinylbenzylammonium, dimethyloctadecylvinylbenzylammonium, glycidyltrimethylammonium, 1-vinyl-3-benzylimidazolium, 1-vinyl-3-hydroxyethylimidazolium or 4-hydroxyethyl-1-vinylpyridinium. Preferred counter ions which can be used include chlorides or other counter ions as disclosed in U.S. Patents 5,223,338, 5,354,813, and 5,403,955. Other mordants suitable for the invention are cationic modified products of polymers such as poly(vinyl alcohol), gelatin, chitosan, polyvinylamine, polyethylene-imine, polydimethyldiallyl ammonium chloride, polyalkylene-polyamine dicyandiamide ammonium condensate, polyvinylpyridinium halide, polymers of (meth)acryloyl oxyalkyl quaternary ammonium salt, polymers of (meth)acrylamide alkyl quaternary ammonium salt, ω-chloro-poly(oxyethylene-polymethylene quaternary ammonium alkylate), methyl glycol chitosan, poly(vinylpyridine), propylene oxide based triamines of the Jeffamine T series, made by Texaco, Inc., quaternary acrylic copolymer latexes, phosphonium compounds, sulfonimides, sulfonated polymers and dispersed particles, and alumina hydrate. Other mordants suitable for the invention are polymers, copolymers, or latexes containing carboxylic acid, sulfonic acid, sulfonamide, sulfonimide, or phosphonic acid, such as carboxylated and sulfonated acrylates or methacrylates, carboxylated styrene butadienes, sulfonated nylons, polyesters and polyurethanes, and their salts. In a preferred embodiment of this invention, the mordanting unit may be chemically incorporated within the chemical structure of the polyester bead. For example, a sulfonated monomer within the polyester structure may serve as a mordant for cationic dye species.

In addition to the ink receiving layers, the recording element may also contain other base layers, next to the support, the function of which is to absorb the solvent from the ink. Materials useful for this layer include inorganic particles and polymeric binder, or highly swellable polymers such as gelatin, sulfonated polyester or poly(vinyl alcohol).

The support for the ink recording element used in the invention can be any of those usually used for inkjet receivers. The support can be either transparent or opaque. Opaque supports include plain paper, coated paper, resin-coated paper such as polyolefin-coated paper, synthetic paper, photographic paper support, melt-extrusion-coated paper, and polyolefin-laminated paper, such as biaxially oriented support laminates. Biaxially oriented support laminates are described in U.S. Patents 5,853,965, 5,866,282, 5,874,205, 5,888,643, 5,888,681, 5,888,683, and 5,888,714. These biaxially oriented supports include a paper base and a biaxially oriented polyolefin sheet, typically polypropylene, laminated to one or both sides of the paper base. The support can also consist of microporous materials such as polyethylene polymer-containing material sold by PPG Industries, Inc., Pittsburgh, Pennsylvania under the trade name of Teslin®, Tyvek® synthetic paper (DuPont Corp.), impregnated paper such as Duraform®, and OPPalyte® films (Mobil Chemical Co.) and other composite films listed in U.S. Patent 5,244,861. Transparent supports include glass, cellulose derivatives, such as a cellulose ester, cellulose triacetate, cellulose diacetate, cellulose acetate propionate, cellulose acetate butyrate, polyesters, such as poly(ethylene terephthalate), poly(ethylene naphthalate), poly-1,4-cyclohexanedimethylene terephthalate, poly(butylene terephthalate), and copolymers thereof, polyimides, polyamides, polycarbonates, polystyrene, polyolefins, such as polyethylene or polypropylene, polysulfones, polyacrylates, polyether imides, and mixtures thereof. The papers listed above include a broad range of papers, from high end papers, such as photographic paper to low end papers, such as newsprint. In a preferred embodiment, Ektacolor paper made by Eastman Kodak Co. is employed. The term as used herein, "transparent" means the ability to pass radiation without significant deviation or absorption.

The support used in the invention may have a thickness of from 50 to 500 µm, preferably from 75 to 300 µm. Antioxidants, brightening agents, antistatic agents, plasticizers and other known additives may be incorporated into the support, if desired.

In order to improve the adhesion of the ink receiving layer to the support, an under-coating or subbing layer may be applied to the surface of the support. This layer may be an adhesive layer such as, for example, halogenated phenols, partially hydrolyzed vinyl chloride-co-vinyl acetate polymer, vinylidene chloride-methyl acrylate-itaconic acid terpolymer, a vinylidene chloride-acrylonitrile-acrylic acid terpolymer, or a glycidyl (meth)acrylate polymer or copolymer. Other chemical adhesives, such as polymers, copolymers, reactive polymers or copolymers, that exhibit good bonding between the ink receiving layer and the support can be used. The polymeric binder in the subbing layer employed in the invention is preferably a water soluble or water dispersible polymer such as poly(vinyl alcohol), poly(vinyl pyrrolidone), gelatin, a cellulose ether, a poly(oxazoline), a poly(vinylacetamide), partially hydrolyzed poly(vinyl acetate/vinyl alcohol), poly(acrylic acid), poly(acrylamide), poly(alkylene oxide), a sulfonated or phosphated polyester or polystyrene, casein, zein, albumin, chitin, chitosan, dextran, pectin, a collagen derivative, collodian, agar-agar, arrowroot, guar, carrageenan, tragacanth, xanthan, rhamsan; a latex such as poly(styrene-co-butadiene), a polyurethane latex, a polyester latex, or a poly(acrylate), poly(methacrylate), poly(acrylamide) or copolymers thereof.

In a preferred embodiment, the subbing layer polymeric binder is a sulfonated polyester dispersion, such as AQ29 ® (Eastman Chemical Co.), gelatin, a polyurethane or poly(vinyl pyrrolidone). The polymeric binder for the subbing layer is preferably used in an amount of from 1 to 50 g/m², preferably from 1 to 20 g/m².

A borate or borate derivative employed in the subbing layer of the ink jet recording element of the invention may be, for example, borax, sodium tetraborate, boric acid, phenyl boronic acid, or butyl boronic acid. As noted above, the borate or borate derivative may be used in an amount of from 3 to 50 g/m², preferably from 3 to 10 g/m². It is believed that upon coating, the borate or borate derivative in the subbing layer diffuses into the image-receiving layer to cross-link the cross-linkable binder in the image-receiving layer.

Other methods to improve the adhesion of the layer to the support include surface treatment of the support by corona-discharge, plasma-treatment in a variety of atmospheres, UV treatment, which may be performed prior to applying the layer to the support.

The recording element utilized in the invention can contain one or more conducting layers such as an antistatic layer to prevent undesirable static discharges during manufacture and printing of the image. This may be added to either side of the element. Antistatic layers conventionally used for color films have been found to be satisfactory, such as those in U.S. Patent 5,147,768. Preferred antistatic agents include metal oxides, e.g., tin oxide, antimony doped tin oxide and vanadium pentoxide. These antistatic agents are preferably dispersed in a film-forming binder.

The layers described above may be coated by conventional coating means onto a support material commonly used in this art. Coating methods may include, but are not limited to, wound wire rod coating, knife coating, slot coating, slide hopper coating, gravure coating, spin coating, dip coating, skim-pan-air-knife coating, multilayer slide bead, doctor blade coating, gravure coating, reverse-roll coating, curtain coating, multilayer curtain coating. Some of these methods allow for simultaneous coatings of more than one layer, which may be preferred from a manufacturing economic perspective if more than one layer or type of layer needs to be applied. Known coating and drying methods are described in further detail in Research Disclosure no. 308119, published Dec. 1989, pages 1007 to 1008. Slide coating may be preferred, in which several layers may be simultaneously applied. The support may be stationary, or may be moving so that the coated layer may be immediately drawn into drying chambers. After coating, the layers may be generally dried by simple evaporation, which may be accelerated by known techniques such as convection heating.

The coating composition may be applied to one or both substrate surfaces through conventional pre-metered or post-metered coating methods listed above. The choice of coating process would be determined from the economics of the operation and in turn, would determine the formulation specifications such as coating solids, coating viscosity, and coating speed. After coating, the ink recording element may be subject to calendering or supercalendering to enhance surface smoothness. In a preferred embodiment of the invention, the ink recording element is subject to hot soft-nip calendering at a temperature of 65°C and a pressure of 14000 kg/m at a speed of from 0.15 m/s to 0.3 m/s.

Inkjet inks used to image the recording elements of the present invention are well known in the art. The ink compositions used in inkjet printing typically may be liquid compositions comprising a solvent or carrier liquid, dyes or pigments, humectants, organic solvents, detergents, thickeners, preservatives. The solvent or carrier liquid can be solely water or can be water mixed with other water-miscible solvents such as polyhydric alcohols. Inks in which organic materials such as polyhydric alcohols are the predominant carrier or solvent liquid may also be used. Particularly useful are mixed solvents of water and polyhydric alcohols. The dyes used in such compositions are typically water-soluble direct or acid type dyes. Such liquid compositions have been described extensively in the prior art including, for example, U.S. Patents 4,381,946, 4,239,543 and 4,781,758.

Used herein, the phrase 'imaging element' comprises an imaging support as described above along with an image receiving or recording layer as applicable to multiple techniques governing the transfer of an image onto the imaging element. Such techniques include thermal dye transfer with thermosensitive imaging materials, electrophotographic printing, or inkjet printing, as well as a support for photographic silver halide images. As used herein, the phrase "photographic element" is a material that utilizes photosensitive silver halide in the formation of images. The stabilized particle of the present invention may be used in a single technique or may be used in a hybrid system combining one or more technique. An example of a hybrid system might be an inkjet printing application on a photographic element.

The thermal ink or dye image-receiving or recording layer of the receiving or recording elements of the invention may comprise, for example, a polycarbonate, a polyurethane, a polyester, polyvinyl chloride, poly(styrene-co-acrylonitrile), poly(caprolactone), or mixtures thereof. The ink or dye image-receiving or recording layer may be present in any amount that is effective for the intended purpose. An overcoat layer may be further coated over the ink or dye-receiving or recording layer, such as described in U.S. Patent No. 4,775,657 of Harrison et al.

Ink or dye-donor elements that may be used with the ink or dye-receiving or recording element of the invention conventionally comprise a support having thereon an ink or dye containing layer. Any ink or dye can be used in the ink or dye-donor employed in the invention, provided it is transferable to the ink or dye-receiving or recording layer by the action of heat. Ink or dye donors applicable for use in the present invention are described, e.g., in U.S. Patent Nos. 4,916,112, 4,927,803, and 5,023,228. As noted above, ink or dye-donor elements may be used to form an ink or dye transfer image. Such a process comprises image-wise-heating an ink or dye-donor element and transferring an ink or dye image to an ink or dye-receiving or recording element as described above to form the ink or dye transfer image. The thermal ink or dye transfer method of printing, an ink or dye donor element may be employed which compromises a poly(ethylene terephthalate) support coated with sequential repeating areas of cyan, magenta, and yellow ink or dye, and the ink or dye transfer steps may be sequentially performed for each color to obtain a three-color ink or dye transfer image. When the process is only performed for a single color, then a monochrome ink or dye transfer image may be obtained.

Thermal printing heads which can be used to transfer ink or dye from ink or dye-donor elements to receiving or recording elements of the invention are available commercially. There can be employed, for example, a Fujitsu Thermal Head (FTP-040 MCS001), a TDK Thermal Head F415 HH7-1089, or a Rohm Thermal Head KE 2008-F3. Alternatively, other known sources of energy for thermal ink or dye transfer may be used, such as lasers as described in, for example, GB No. 2,083,726A.

A thermal ink or dye transfer assemblage may comprise (a) an ink or dye-donor element, and (b) an ink or dye-receiving or recording element as described above, the ink or dye-receiving or recording element being in a superposed relationship with the ink or dye-donor element so that the ink or dye layer of the donor element may be in contact with the ink or dye image-receiving or recording layer of the receiving or recording element.

When a three-color image is to be obtained, the above assemblage may be formed on three occasions during the time when heat is applied by the thermal printing head. After the first dye is transferred, the elements may be peeled apart. A second dye-donor element (or another area of the donor element with a different dye area) may be then brought in register with the dye-receiving or recording element and the process repeated. The third color may be obtained in the same manner.

The electrographic and electrophotographic processes and their individual steps have been well described in the prior art. The processes incorporate the basic steps of creating an electrostatic image, developing that image with charged, colored particles (toner), optionally transferring the resulting developed image to a secondary substrate, and fixing the image to the substrate. There are numerous variations in these processes and basic steps, the use of liquid toners in place of dry toners is simply one of those variations.

The first basic step, creation of an electrostatic image, can be accomplished by a variety of methods. In one form, the electrophotographic process of copiers uses imagewise photodischarge, through analog or digital exposure, of a uniformly charged photoconductor. The photoconductor may be a single-use system, or it may be rechargeable and reimageable, like those based on selenium or organic photoreceptors.

In an alternate electrographic process, electrostatic images may be created ionographically. The latent image may be created on dielectric (charge-holding) medium, either paper or film. Voltage may be applied to selected metal styli or writing nibs from an array of styli spaced across the width of the medium, causing a dielectric breakdown of the air between the selected styli and the medium. Ions may be created, which form the latent image on the medium.

Electrostatic images, however generated, may be developed with oppositely charged toner particles. For development with liquid toners, the liquid developer may be brought into direct contact with the electrostatic image. Usually a flowing liquid is employed to ensure that sufficient toner particles are available for development. The field created by the electrostatic image causes the charged particles, suspended in a nonconductive liquid, to move by electrophoresis. The charge of the latent electrostatic image may be thus neutralized by the oppositely charged particles. The theory and physics of electrophoretic development with liquid toners are well described in many books and publications.

If a reimageable photoreceptor or an electrographic master is used, the toned image may be transferred to paper (or other substrate). The paper may be charged electrostatically, with the polarity chosen to cause the toner particles to transfer to the paper. Finally, the toned image may be fixed to the paper. For self-fixing toners, residual liquid may be removed from the paper by air-drying or heating. Upon evaporation of the solvent, these toners form a film bonded to the paper. For heat-fusible toners, thermoplastic polymers may be used as part of the particle. Heating both removes residual liquid and fixes the toner to paper.

When used as inkjet imaging media, the recording elements or media typically comprise a substrate or a support material having on at least one surface thereof an ink-receiving or recording / recording or image-forming layer. If desired, in order to improve the adhesion of the inkjet receiving or recording layer to the support, the surface of the support may be corona-discharge-treated prior to applying the solvent-absorbing layer to the support or, alternatively, an undercoating, such as a layer formed from a halogenated phenol or a partially hydrolyzed vinyl chloride-vinyl acetate copolymer, can be applied to the surface of the support. The inkjet receiving or recording layer is preferably coated onto the support layer from water or water-alcohol solutions at a dry thickness ranging from 3 to 75 micrometers, preferably 8 to 50 micrometers.

Any known inkjet receiver layer can be used in combination with other particulate materials. For example, the ink receiving or recording layer may consist primarily of inorganic oxide particles such as silicas, modified silicas, clays, aluminas, fusible beads such as beads comprised of thermoplastic or thermosetting polymers, non-fusible organic beads, or hydrophilic polymers such as naturally-occurring hydrophilic colloids and gums such as gelatin, albumin, guar, xantham, acacia, chitosan, starches and their derivatives, derivatives of natural polymers such as functionalized proteins, functionalized gums and starches, and cellulose ethers and their derivatives, and synthetic polymers such as polyvinyloxazoline, polyvinylmethyloxazoline, polyoxides, polyethers, poly(ethylene imine), poly(acrylic acid), poly(methacrylic acid), n-vinyl amides including polyacrylamide and polyvinylpyrrolidone, and poly(vinyl alcohol), its derivatives and copolymers, and combinations of these materials. Hydrophilic polymers, inorganic oxide particles, and organic beads may be present in one or more layers on the substrate and in various combinations within a layer.

A porous structure may be introduced into ink receiving or recording layers comprised of hydrophilic polymers by the addition of ceramic or hard polymeric particulates, by foaming or blowing during coating, or by inducing phase separation in the layer through introduction of non-solvent. In general, it is preferred for the base layer to be hydrophilic, but not porous. This may be especially true for photographic quality prints, in which porosity may cause a loss in gloss. In particular, the ink receiving or recording layer may consist of any hydrophilic polymer or combination of polymers with or without additives as is well known in the art.

If desired, the ink receiving or recording layer can be overcoated with an ink-permeable, anti-tack protective layer such as, for example, a layer comprising a cellulose derivative or a cationically-modified cellulose derivative or mixtures thereof. An especially preferred overcoat is poly β-1,4-anhydro-glucose-g-oxyethylene-g-(2'-hydroxypropyl)-N,N-dimethyl-N-dodecylammonium chloride. The overcoat layer is non porous, but is ink permeable and serves to improve the optical density of the images printed on the element with water-based inks. The overcoat layer can also protect the ink receiving or recording layer from abrasion, smudging, and water damage. In general, this overcoat layer may be present at a dry thickness of 0.1 to 5 µm, preferably 0.25 to 3 µm.

In practice, various additives may be employed in the ink receiving or recording layer and overcoat. These additives include surface active agents such as surfactant(s) to improve coatability and to adjust the surface tension of the dried coating, acid or base to control the pH, antistatic agents, suspending agents, antioxidants, hardening agents to cross-link the coating, antioxidants, UV stabilizers, light stabilizers. In addition, a mordant may be added in small quantities (2%-10% by weight of the base layer) to improve waterfastness. Useful mordants are disclosed in U.S. Patent No. 5,474,843.

The layers described above, including the ink receiving or recording layer and the overcoat layer, may be coated by conventional coating means onto a transparent or opaque support material commonly used in this art. Coating methods may include, but are not limited to, blade coating, wound wire rod coating, slot coating, slide hopper coating, gravure, curtain coating. Some of these methods allow for simultaneous coatings of both layers, which is preferred from a manufacturing economic perspective.

The IRL (ink or dye receiving layer) may be coated over a tie layer (TL). There arc many known formulations which may be useful as ink or dye receiving or recording layers. The primary requirement is that the IRL is compatible with the inks which it will be imaged so as to yield the desirable color gamut and density. As the ink drops pass through the IRL, the ink or dyes may be retained or mordanted in the IRL, while the ink solvents pass freely through the IRL and may be rapidly absorbed by the TL. Additionally, the IRL formulation is preferably coated from water, exhibits adequate adhesion to the TL, and allows for easy control of the surface gloss.

For example, Misuda et al in US Patents 4,879,166, 5,264,275, 5,104,730, 4,879,166, and Japanese Patents 1,095,091, 2,276,671, 2,276,670, 4,267,180, 5,024,335, and 5,016,517 disclose aqueous based IRL formulations comprising mixtures of psuedo-bohemite and certain water soluble resins. Light in US Patents 4,903,040, 4,930,041, 5,084,338, 5,126,194, 5,126,195, and 5,147,717 discloses aqueous-based IRL formulations comprising mixtures of vinyl pyrrolidone polymers and certain water-dispersible and/or water-soluble polyesters, along with other polymers and addenda. Butters et al in US Patents 4,857,386 and 5,102,717 disclose ink-absorbent resin layers comprising mixtures of vinyl pyrrolidone polymers and acrylic or methacrylic polymers. Sato et al in US Patent 5,194,317 and Higuma et al in US Patent 5,059,983 disclose aqueous-coatable IRL formulations based on poly(vinyl alcohol). Iqbal in US Patent 5,208,092 discloses water-based IRL formulations comprising vinyl copolymers which may be subsequently cross-linked. In addition to these examples, there may be other known or contemplated IRL formulations which are consistent with the aforementioned primary and secondary requirements of the IRL, all of which fall under the spirit and scope of the current invention.

The IRL may also contain varying levels and sizes of matting agents for the purpose of controlling gloss, friction, and/or fingerprint resistance, surfactants to enhance surface uniformity and to adjust the surface tension of the dried coating, mordanting agents, antioxidants, UV absorbing compounds, light stabilizers.

It may also be desirable to overcoat the IRL for the purpose of enhancing the durability of the imaged element. Such overcoats may be applied to the IRL either before or after the element is imaged. For example, the IRL can be overcoated with an ink-permeable layer through which inks freely pass. Layers of this type are described in US Patents 4,686,118, 5,027,131, and 5,102,717. Alternatively, an overcoat may be added after the element is imaged. Any of the known laminating films and equipment may be used for this purpose. The inks used in the aforementioned imaging process are well known, and the ink formulations are often closely tied to the specific processes, i.e., continuous, piezoelectric, or thermal. Therefore, depending on the specific ink process, the inks may contain widely differing amounts and combinations of solvents, colorants, preservatives, surfactants, humectants. Inks preferred for use in combination with the image recording elements of the present invention may be water-based. However, it may be intended that alternative embodiments of the image-recording elements as described above, which may be formulated for use with inks which are specific to a given ink-recording process or to a given commercial vendor, fall within the scope of the present invention.

In another embodiment, in order to produce photographic elements, the composite support sheet may be coated with a photographic element or elements. The photographic elements can be single color elements or multicolor elements. Multicolor elements contain image ink or dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

The photographic emulsions useful for this invention may be generally prepared by precipitating silver halide crystals in a colloidal matrix by methods conventional in the art. The colloid may be typically a hydrophilic film forming agent such as gelatin, alginic acid, or derivatives thereof.

The crystals formed in the precipitation step may be washed and then chemically and spectrally sensitized by adding spectral sensitizing dyes and chemical sensitizers, and by providing a heating step during which the emulsion temperature may be raised, typically from 40.degree. C. to 70.degree. C., and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea, reducing agents, e.g., polyamines and stannous salts, noble metal compounds, e.g., gold, platinum, and polymeric agents, e.g., polyalkylene oxides. As described, heat treatment may be employed to complete chemical sensitization. Spectral sensitization may be effected with a combination of dyes, which are designed for the wavelength range of interest within the visible or infrared spectrum. It is known to add such dyes both before and after heat treatment.

After spectral sensitization, the emulsion may be coated on a support. Various coating techniques include dip coating, air knife coating, curtain coating and extrusion coating.

The silver halide emulsions utilized in this invention may be comprised of any halide distribution. Thus, they may be comprised of silver chloride, silver bromide, silver bromochloride, silver chlorobromide, silver iodochloride, silver iodobromide, silver bromoiodochloride, silver chloroiodobromide, silver iodobromochloride, and silver iodochlorobromide emulsions. By predominantly silver chloride, it is meant that the grains of the emulsion are greater than 50 mole percent silver chloride. Preferably, they are greater than 90 mole percent silver chloride, and optimally greater than 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular or core / shell grains. Grains having a tabular or cubic morphology may be preferred.

Elements of the invention which may contain photographic materials may utilize emulsions as described in The Theory of the Photographic Process, Fourth Edition, T. H. James, Macmillan Publishing Company, Inc., 1977, pages 151-152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions may be added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitize an emulsion include ascorbic acid derivatives, tin compounds, polyamine compounds, and thiourea dioxide-based compounds described in U.S. Pat. Nos. 2,487,850, 2,512,925, and British Patent 789,823. Specific examples of reduction sensitizers or conditions, such as dimethylamineborane, stannous chloride, hydrazine, high pH (pH 8-11) and low pAg (pAg 1-7) ripening are discussed by S. Collier in Photographic Science and Engineering, 23, 113 (1979). Examples of processes for preparing intentionally reduction sensitized silver halide emulsions are described in EP 0 348 934 Al (Yamashita), EP 0 369 491 (Yamashita), EP 0 371 388 (Ohashi), EP 0 396 424 A1 (Takada), EP 0 404 142 Al (Yamada), and EP 0 435 355 A1 (Makino).

The photographic elements of this invention may use emulsions doped with Group VII metals such as iridium, rhodium, osmium, and iron as described in Research Disclosure, September 1994, Item 36544, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," Photographic Science and Engineering, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants may be incorporated, emulsions show an increased fresh fog and a lower contrast sensitometric curve when processed in the color reversal E-6 process as described in The British Journal of Photography Annual, 1982, pages 201-203.

A typical multicolor photographic element comprises the invention laminated support bearing a cyan ink or dye image-forming unit comprising at least one red-sensitive silver halide emulsion layer having associated therewith at least one cyan dye-forming coupler, a magenta image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers. The support may also be utilized for black and white photographic print elements.

The photographic elements may also contain a transparent magnetic recording layer such as a layer containing magnetic particles on the underside of a transparent support, as in U.S. Pat. Nos. 4,279,945 and 4,302,523. The invention may be utilized with the materials disclosed in Research Disclosure, September 1997, Item 40145. The invention may be particularly suitable for use with the material color paper examples of sections XVI and XVII. The couplers of section II are also particularly suitable. The Magenta I couplers of section II, particularly M-7, M-10, M-18, and M-18, set forth below are particularly desirable. In the following Table, reference will be made to (1) Research Disclosure, December 1978, Item 17643, (2) Research Disclosure, December 1989, Item 308119, and (3) Research Disclosure, September 1994, Item 36544, all published by Kenneth Mason Publications, Ltd., Dudley Annex, 12a North Street, Emsworth, Hampshire PO10 7DQ, ENGLAND. The Table and the references cited in the Table are to be read as describing particular components suitable for use in the elements of the invention. The Table and its cited references also describe suitable ways of preparing, exposing, processing and manipulating the elements, and the images contained therein.

| Reference | | | |
|---|---|---|---|
| | Section | Subject Matter | |
| 1 | I, II | Grain composition, | |
| 2 | I, II, IX, X, XI, | morphology and preparation. | |
| | XII, XIV, XV | Emulsion preparation including | |
| | I, II, III, IX | hardeners, coating aids, | |
| 3 | A & B | addenda | |
| 1 | III, IV | Chemical sensitization and | |
| 2 | III, IV | spectral sensitization | |
| 3 | IV, V | Desensitization. | |
| 1 | V UV | dyes, optical brighteners, | |
| 2 | V | luminescent dyes | |
| 3 | VI | | |
| 1 | VI | Antifoggants and stabilizers | |
| 2 | VI | | |
| 3 | VII | | |
| 1 | VIII | Absorbing and scattering | |
| 2 | VIII, XIII, XVI | materials; Antistatic layers; | |
| 3 | VIII, IX C & D | matting agents | |
| 1 | VII | Image-couplers and image- | |
| | 2 | VII | modifying couplers; Dye |
| | 3 | X | stabilizers and hue modifiers |
| | 1 | XVII | Supports |
| | 2 | XVII | |
| | 3 | XV | |
| | 3 | XI | Specific layer arrangements |
| | 3 | XII, XIII | Negative working emulsions; Direct positive emulsions |
| | 2 | XVIII | Exposure |
| | 3 | XVI | |
| | I | XIX, XX | Chemical processing; |
| | 2 | XIX, XX, XXII | Developing agents |
| | 3 | XVIII, XIX, XX | |
| | 3 | XIV | Scanning and digital processing procedures |

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible image, preferably by other than heat treatment. Processing may be preferably carried out in the known RA-4.TM. (Eastman Kodak Company) Process or other processing systems suitable for developing high chloride emulsions. This invention is also directed towards a photographic recording element comprising a support and at least one light sensitive silver halide emulsion layer comprising silver halide grains as described above.

Although the recording elements disclosed herein have been referred to primarily as being useful for inkjet printers, they also can be used as recording media for pen plotter assemblies. Pen plotters operate by writing directly on the surface of a recording medium using a pen consisting of a bundle of capillary tubes in contact with an ink reservoir.

The following examples are intended to further illustrate, but not to limit, the invention.

### EXAMPLES

### Preparation of porous polyester particles PE-1 through PE-4

Precursor polyesters PP-1 through PP-3 were all synthesized by a 2-stage melt polycondensation process. The chemical compositions are listed in Table 1 and the reaction times and final molecular weights are listed in Table 2. The SIP, CHDM, dibutylstannoic acid, zinc acetate, and sodium acetate were combined in a 500 ml 3-neck flask equipped with a stainless steel stirring rod, nitrogen inlet, and an arm leading to a dry ice/acetone condenser with an outlet connected to a controlled vacuum system. A graduated cylinder was connected beneath the condenser with a ground glass joint to collect and measure distillate. The reaction was heated in a thermostatted bath containing a metal heating alloy. A steady stream of nitrogen was passed over the reaction mixture for 10 minutes, and was then reduced to a slightly positive flow. The temperature was held at 210-230°C for 100-250 minutes with stirring at~100 RPM until a clear prepolymer resulted and the calculated amount of methanol distillate had been collected in a graduated cylinder. The reaction was removed from the bath and allowed to cool. The FA and IPA were then added and the condenser was filled with ice. The reaction was restarted at 220°C and within 20 minutes water condensate began to collect. The reaction was held at 220°C for 130-460 minutes until the viscosity of the melt had increased to the point where the polyester could no longer be effectively stirred and the reaction was terminated.

**Table 1**

| | **FA (g)** | **SIP (g)** | **IPA (g)** | **Mol ratio FA:SIP:IPA** | **CHDM (g)** | **Zn(OAc)₂ (g)** | **BuSn(OH)₃ (g)** | **NaOAc (g)** |
|---|---|---|---|---|---|---|---|---|
| PP-1 | 19.59 | 50.01 | - | 1:1:0 | 45.57 | 0.02 | 0.02 | 0.69 |
| PP-2 | 21.43 | 27.35 | 15.34 | 2:1:1 | 51.13 | 0.02 | 0.02 | 0.38 |
| PP-3 | 48.99 | 125.02 | - | 1:1:0 | 116.42 | 0.06 | 0.04 | 1.73 |

| | | | | | | | | |
|---|---|---|---|---|---|---|---|---|
| FA is fumaric acid SIP is dimethyl 5-sulfoisophthalate, sodium salt IPA is isophthalic acid CHDM is 1,4-cyclohexanedimethanol, mixture *of cis* and *trans* isomers. | | | | | | | | |

**Table 2**

| | **Stage 1 reaction time** | **Stage 2 reaction time** | **Mn** | **Mw** |
|---|---|---|---|---|
| PP-1 | 120 min | 130 min | 2,710 | 10,500 |
| PP-2 | 100 min | 420 min | 3,570 | 15,800 |
| PP-3 | 250 min | 200 min | 3,240 | 7,330 |

Precursor polyester PP-4 was synthesized using the same apparatus as used above for PP-1 through PP-3, and a similar 2-stage procedure. In the first stage, SIP (82.41 g, 0.28 mol), hydroquinone-bis-hydroxyethyl ether (HQBHE) (110.29 g, 0.56 mol), sodium acetate (2.28 g), and titanium isopropoxide (4 drops) were combined in a 500 ml 3-neck round bottom flask and heated for 220-240°C for 70 minutes at which point a clear, slightly orange prepolymer had formed and the calculated amount of methanol condensate had been collected. The reaction was then cooled and diethyl fumarate (47.90 g, 0.28 mol) was added. The reaction was restarted and was heated at 200°C for 100 minutes followed by 120 minutes at 220°C. A vacuum was then initiated which ramped from ambient pressure to 20 torr over 2 minutes. The viscosity of the melt began to rapidly increase and the reaction was terminated. (Mn = 2940, Mw = 5440).

Polyester particles PE-1 through PE-4 were all synthesized by the following procedure. An aqueous phase was prepared by dispersing appropriate precursor polyester in the amount of water noted in Table 3. The water generally had to be heated to 40-60°C and it required from 20 minutes to 16 hours for the precursor polyester to completely disperse, depending on the amount of SIP monomer in the precursor polyester. The aqueous phase was filtered through cheesecloth and combined in a beaker with an organic phase consisting of the toluene, DVB, hexadecane, and AIBN. The 2 phases were emulsified by any of the three methods listed in Table 3 and transferred to an appropriately sized 3-neck 1 L round bottom flask fitted with a mechanical stirrer and a reflux condenser with nitrogen inlet. The opaque white microsuspensions were bubble degassed with nitrogen for 10 minutes, then heated overnight at 70°C for 16 hours. The resulting particle dispersions were cooled to room temperature and the toluene was removed as a water azeotrope via rotary evaporation. The dispersions were washed with 4-6 volumes of water and concentrated to 9-25% solids using a Millipore Amicon ultrafiltration system with a 100K cutoff spiral-wound dialysis cartridge. The exact concentrations of each PE dispersion are listed in Table 4.

**Table 3**

| **Disper sion** | **Precursor polyester** | **Precursor polyester (g)** | **Water (ml)** | **DVB¹ (g)** | **Toluene (g)** | **AIBN ⁴ (g)** | **Hexadecane (ml)** | **Emulsification method** |
|---|---|---|---|---|---|---|---|---|
| PE-1 | PP-1 | 20.00 | 240 | 20.00 | 40.00 | 0.40 | 4.14 | M² |
| PE-2 | PP-2 | 20.00 | 240 | 20.00 | 40.00 | 0.40 | 4.14 | M² |
| PE-3 | PP-3 | 62.50 | 750 | 68.38 | 125.00 | 1.25 | 12.94 | H³ |
| PE-4 | PP-4 | 40.00 | 514 | 40.0 | 80.0 | 0.80 | 2.82 | H³ |
| PE-5 | PP-4 | 25.25 | 122 | 20.25 | 0 | 0.41 | 0.81 | H³ |

| | | | | | | | | |
|---|---|---|---|---|---|---|---|---|
| ¹ DVB is divinylbenzene (80% w/w with remainder being ethyl styrene, mixture of *m* and p isomers.) ² Reaction mixture was passed twice through an M-110T Microfluidizer (sold by Microfluidics). ³ Reaction mixture was homogenized for 10 minutes using a Silverson L4 mixer on the highest setting. ⁴ AIBN is 2,2'-azobis(isobutyronitrile) | | | | | | | | |

### Determination of particle size and particle size distribution

The particle size and particle size distribution of each particle was measured using a laser scattering particle size distribution analyzer, Horiba LA-920, manufactured by Horiba LTD. The results for PE-1 through PE-4 are in Table 4.

**Table 4**

| **PE dispersion** | **Wt% solids** | **Mode 1** | | | **Mode 2** | | |
|---|---|---|---|---|---|---|---|
| | | **Mean diameter (micron)** | **Proportion (%)** | **CV (%)** | **Mean diameter (micron)** | **Proportion (%)** | **CV %** |
| PE-1 | 13.54 | 0.356 | 100 | 35.2 | -- | -- | -- |
| PE-2 | 12.97 | 0.181 | 5.9 | 15.9 | 0.351 | 94.1 | 36.8 |
| PE-3 | 22.86 | 1.082 | 9.1 | 44.2 | 2.69 | 90.9 | 27.1 |
| PE-4 | 17.60 | 0.434 | 27.6 | 45.3 | 4.46 | 72.4 | 57.5 |

### Example 1

### Preparation of Control Element C-1 (single layer of larger size particles)

A coating composition was prepared from 53.92 wt. % of dispersion PE-3, 2.18 wt. % poly(vinyl alcohol), PVA, (Gohsenol® GH-17 from Nippon Gohsei Co., Ltd.), and 43.90 wt. % water. [The relative proportions of porous polyester particle to PVA are therefore 85/15 by weight]. The coating composition was metered to a slot-die coating apparatus and coated onto a base support comprised of a polyethylene resin coated photographic paper stock, which had previously been subjected to corona discharge treatment, moving at a speed of about 2.4 m/min. The coated support immediately entered the drying section of the coating machine to remove substantially all solvent components and form an ink receiving layer. The thickness of the dry ink receiving layer was measured to be about 15 ± 2 µm. The measured surface gloss, print density of the cyan patch at Dmax, and the ink dry time are reported in Table 5.

### Preparation of Element 1

A coating composition (Solution S-3) was prepared the same as in Control Element C-1. A second coating composition (Solution S-1) was prepared from 62.78 wt. % of dispersion PE-1, 1.5 wt. % poly(vinyl alcohol), PVA, (Gohsenol® GH-17 from Nippon Gohsei Co., Ltd.), and 35.72 wt. % water. [The relative proportions of porous polyester particle to PVA are therefore 85/15 by weight]. Both coating compositions were metered to a multiple-slot-die coating apparatus and coated simultaneously, with Solution S-3 being located below (closer to the support than) Solution S-1, onto a base support comprised of a polyethylene resin coated photographic paper stock, which had previously been subjected to corona discharge treatment, moving at a speed of about 2.4 m/min. The coated support immediately entered the drying section of the coating machine to remove substantially all solvent components and form a two-layer image receiving element. The combined thickness of the dry ink receiving layers was measured to be about 19 ± 2 µm. The measured surface gloss, print density of the cyan patch at Dmax, and the ink dry time are reported in Table 5.

### Preparation of Element 2

Coating compositions S-3 and S-1 were prepared the same as Element 1 except that Solution S-1 was 59.08 wt. % of dispersion PE-1, 2.0 wt. % poly(vinyl alcohol), PVA, (Gohsenol® GH-17 from Nippon Gohsei Co., Ltd.), and 38.92 wt. % water. [The relative proportions of porous polyester particle to PVA are therefore 80/20 by weight]. The coating composition were coated and dried the same as Element 1, with Solution S-3 being located below (closer to the support than) Solution S-1. The combined thickness of the dry ink receiving layers was measured to be about 20 ± 2 µm. The measured surface gloss, print density of the cyan patch at Dmax, and the ink dry time are reported in Table 5.

### Preparation of Element 3

A coating composition (Solution S-3) was prepared the same as in Control Element C-1. A second coating composition (Solution S-2) was prepared from 65.54 wt. % of dispersion PE-2, 1.5 wt. % poly(vinyl alcohol), PVA, (Gohsenol® GH-17 from Nippon Gohsei Co., Ltd.), and 32.96 wt. % water. [The relative proportions of porous polyester particle to PVA are therefore 85/15 by weight]. The coating compositions were coated and dried the same as Element 1, with Solution S-3 being located below (closer to the support than) Solution S-2. The thickness of the dry lower layer was measured to be about 12 ± 2 µm and the thickness of the dry upper layer was measured to be about 9 ± 2 µm. The measured surface gloss, print density of the cyan patch at Dmax, and the ink dry time are reported in Table 5.

### Preparation of Element 4

Coating compositions S-3 and S-2 were prepared, coated and dried the same as Element 3 except that the thickness of the layers were different. The combined thickness of the dry ink receiving layers was measured to be about 12 ± 2 µm. The measured surface gloss, print density of the cyan patch at Dmax, and the ink dry time are reported in Table 5.

### Preparation of Element 5

A coating composition (Solution S-3) was prepared the same as in Control Element C-1. A second coating composition S-4 was prepared from 48.30 wt. % of dispersion PE-4, 1.5 wt. % poly(vinyl alcohol), PVA, (Gohsenol® GH-17 from Nippon Gohsei Co., Ltd.), and 50.20 wt. % water. [The relative proportions of porous polyester particle to PVA are therefore 85/15 by weight]. The coating composition were coated and dried the same as Element 1, with Solution S-3 being located below (closer to the support than) Solution S-4. The thickness of the dry lower layer was measured to be about 20 ± 2 µm and the thickness of the dry upper layer was measured to be about 5 ± 2 µm. The measured surface gloss, print density of the cyan patch at Dmax, and the ink dry time are reported in Table 5.

### Printing

The above elements and control elements of Example 1 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) were read using an X-Rite ® 820 densitometer. The cyan density is reported in Table 5.

### Surface gloss measurement

The gloss of the top surface of the unprinted ink receiving layer was measured using a BYK Gardner gloss meter at an angle of illumination/reflection of 60°. The results are related to a highly polished black glass with a refractive index of 1.567 that has a specular gloss value of 100. The results are reported in Table 5.

### Measurement of ink dry time

A drop (from a 10 microliter capillary tube) of a magenta inkjet ink, prepared using a standard formulation with Dye 6 from U.S. Patent 6,001,161, was placed on each unprinted element and the time that it took for this spot to become dry to the touch was measured as the "ink drying time" as shown in Table 5.

**Table 5**

| **Element** | **Cyan D-max** | **60° gloss** | **Ink drying time (seconds)** |
|---|---|---|---|
| 1 | 1.7 | 23 | 100 |
| 2 | 1.6 | 30 | 120 |
| 3 | 1.7 | 65 | 120 |
| 4 | 1.7 | 48 | 180 |
| 5 | 1.6 | 10 | 20 |
| Control C-1 | 1.1 | 3 | > 180 |

The above results show that higher surface gloss and improved print density for the element can be achieved with a multilayer ink receiving layer structure when the upper layer contains porous polyester particles that have a mean diameter of less than 0.5 micrometers.

### Example 2

### Synthesis of core-shell latex dispersion D-1

The core-shell latex employed in this invention was prepared by a sequential emulsion polymerization technique in which the core polymer latex is polymerized first, followed by the sequential feeding of a second monomer suspension. The following reagents were used in this synthesis.

| | |
|---|---|
| A: | Deionized water (50 g) |
| | Triton 770® (30% active) (0.4 g) |
| B: | Potassium persulfate (0.12 g) |
| C: | Methyl methacrylate (17.1 g) |
| | Sodium 2-sulfo-1,1-dimethylethyl acrylamide (0.9 g) |
| | Potassium persulfate (0.1 g) |
| | Triton 770® (30% active) (0.9g) |
| | Deionized water (35 g) |
| D: | Ethyl acrylate (3.6 g) |
| | Vinylidene chloride (31.0 g) |
| | Sodium 2-sulib-1,1-dimethylethyl acrylamide (1.44 g) |
| | Potassium persulfate (0.21 g) |
| | Sodium bisulfate (0.42 g) |
| | Triton 770® (30% active) (5.80 g) |
| | Deionized water (160 g) |

Reagent combination A was charged to a 1L 3-neck flask equipped with a nitrogen inlet, mechanical stirrer and condenser. The flask was immersed in a constant temperature bath at 80 °C and purged with nitrogen for 20 min. Reagent B was added and followed by the addition of reagent mixture C over 2 hours. The mixture (C) was agitated with constant agitation to keep the mixture in the form of a suspension. The polymerization was continued for 30 min and the latex was cooled to 40 °C. The second monomer suspension (D) was prepared and added in the same way. The total addition time was two hours. The latex was heated at 40 °C for one additional hour and 4 ml of 10 wt. % t-butyl hydroperoxide and 10 wt. % formaldehyde-sulfite were added to remove the residual monomer. The reaction was held for 30 min, cooled to room temperature and filtered, resulting in dispersion D-1.

The latex dispersion had a pH = 2.0 and was adjusted to a pH = 6.0 by adding a few drops of a dilute solution of sodium hydroxide. The concentration of the aqueous dispersion was 16.74 wt. % solids. The mean diameter of the particles was measured to be 117 nanometers.

### Preparation of Element 6

A coating composition (Solution S-3) was prepared the same as in Control Element C-1. A second coating composition (Solution S-5) was prepared from 50.8 wt. % of dispersion D-1, 1.5 wt. % poly(vinyl alcohol), PVA, (Gohsenol® GH-17 from Nippon Gohsei Co., Ltd.), and 47.7 wt. % water. [The relative proportions of organic polymer particle to PVA are therefore 85/15 by weight]. Both coating compositions were metered to a multiple-slot-die coating apparatus and coated simultaneously, with Solution S-3 being located below (closer to the support than) Solution S-5, onto a base support comprised of a polyethylene resin coated photographic paper stock, which had been previously subjected to corona discharge treatment, moving at a speed of about 2.4 m/min. The coated support immediately entered the drying section of the coating machine to remove substantially all solvent components and form a two-layer image receiving element. The combined thickness of the dry ink receiving layers was measured to be about 26 ± 2 µm. The element was printed the same as in Example 1. The surface gloss and print density of the cyan patch at Dmax were measured the same as in Example 1 and the results are reported in Table 6.

### Synthesis of non-porous polyester particle

Non-porous polymer particle PE-5 were synthesized by the same procedure used for PE-1 through PE-4 except that the toluene component was not added, and thus the azeotropic removal step was not needed. The concentration of the aqueous dispersion was 12.78 wt. % solids. The mean diameter of the particles was measured to be 307 nanometers.

### Preparation of Element 7

A coating composition (Solution S-3) was prepared the same as in Control Element C-1. A second coating composition (Solution S-6) was prepared from 66.5 wt. % of polyester particle PE-5, 1.5 wt. % poly(vinyl alcohol), PVA, (Gohsenol® GH-17 from Nippon Gohsei Co., Ltd.), and 32.0 wt. % water. [The relative proportions of polyester particle to PVA are therefore 85/15 by weight]. Both coating compositions were metered to a multiple-slot-die coating apparatus and coated simultaneously, with Solution S-3 being located below (closer to the support than) Solution S-6, onto a base support comprised of a polyethylene resin coated photographic paper stock, which had been previously subjected to corona discharge treatment, moving at a speed of about 2.4 m/min. The coated support immediately entered the drying section of the coating machine to remove substantially all solvent components and form a two-layer image receiving element. The combined thickness of the dry ink receiving layers was measured to be about 28 ± 2 µm. The element was printed the same as in Example 1. The surface gloss and print density of the cyan patch at Dmax were measured the same as in Example 1 and the results are reported in Table 6.

### Preparation of Element 8

A coating composition (Solution S-3) was prepared, coated, and dried the same as in Control Element C-1, forming layer L-1. A second coating composition (Solution S-7) was prepared from 55.2 wt. % of colloidal silica solution TX-11005 (30.8 wt % silica in water, listed particle size is 118 nanometers, from Nalco Chemical Company), 3.0 wt. % poly(vinyl alcohol), PVA, (Gohsenol® GH-17 from Nippon Gohsei Co., Ltd.), and 41.8 wt. % water. [The relative proportions of silica particle to PVA are therefore 85/15 by weight]. Solution S-7 was coated over the layer L-1 using a calibrated coating knife, and dried to remove substantially all solvent components to form layer L-2. The thickness of layer L-1 was measured to be about 15 ± 2 µm, and the thickness of layer L-2 was measured to be about 3 ± 2 µm. The element was printed the same as in Example 1. The surface gloss and print density of the cyan patch at Dmax were measured the same as in Example 1 and the results are reported in Table 6.

### Preparation of Element 9

A coating composition (Solution S-3) was prepared, coated, and dried the same as in Control Element C-1, forming layer L-1. A second coating composition (Solution S-8) was prepared from 42.5 wt. % of a fumed alumina solution (40 wt. % alumina in water, Cab-O-Sperse® PG003 from Cabot Corporation), 1.8 wt. % poly(vinyl alcohol), PVA, (Gohsenol® GH-17 from Nippon Gohsei Co., Ltd.), 0.8 wt % of 2,3-dihydroxy-1,4-dioxane (Clariant Corp.), and 54.9 wt. % water. Solution S-8 was coated over the layer L- 1 using a calibrated coating knife, and dried to remove substantially all solvent components to form layer L-3. The thickness of layer L-1 was measured to be about 15 ± 2 µm, and the thickness of layer L-3 was measured to be about 3 ± 2 µm. The element was printed the same as in Example 1. The surface gloss and print density of the cyan patch at Dmax were measured the same as in Example 1 and the results are reported in Table 6.

### Preparation of Element 10

A coating composition (Solution S-3) was prepared, coated, and dried the same as in Control Element C-1, forming layer L-1. A second coating composition (Solution S-9) was prepared from 100 wt. % of Viviprint 540 (10 wt % polyvinylpyrrolidone hydrogel in water from International Specialty Products). Solution S-9 was coated over the layer L-1 using a calibrated coating knife, and dried to remove substantially all solvent components to form layer L-4. The thickness of layer L-1 was measured to be about 15 ± 2 µm, and the thickness of layer L-4 was measured to be about 4 ± 2 µm. The element was printed the same as in Example 1. The surface gloss and print density of the cyan patch at Dmax were measured the same as in Example 1 and the results are reported in Table 6.

### Preparation of Element 11

A coating composition (Solution S-3) was prepared, coated, and dried the same as in Control Element C-1, forming layer L-1. A second coating composition (Solution S-10) was prepared from 10 wt. % poly(vinyl alcohol), PVA, (Airvol 2035 from Air Products and Chemicals, Inc.) and 90 wt. % water. Solution S-10 was coated over the layer L-1 using a calibrated coating knife, and dried to remove substantially all solvent components to form layer L-5. The thickness of layer L-1 was measured to be about 15 ± 2 µm, and the thickness of layer L-5 was measured to be about 1 ± 0.5 µm. The element was printed the same as in Example 1. The surface gloss and print density of the cyan patch at Dmax were measured the same as in Example 1 and the results arc reported in Table 6.

**Table 6**

| **Element** | **Particle in lower ink receiving layer** | **Particle in upper ink receiving layer** | **Cyan D-max** | **60° gloss** |
|---|---|---|---|---|
| 6 | PE-3 | D-1 | 1.7 | 21 |
| 7 | PE-3 | PE-5 | 1.6 | 44 |
| 8 | PE-3 | TS-11005 silica | 1.6 | 10 |
| 9 | PE-3 | Fumed alumina | 2.0 | 25 |
| 10 | PE-3 | none | 2.0 | 41 |
| 11 | PE-3 | none | 1.9 | 15 |

The above results show that higher surface gloss and improved print density for the element can be achieved, relative to those obtained with control element C-1, with a multilayer ink receiving layer structure, particularly when the upper layer contains organic or inorganic particles that have a mean diameter of less than 0.5 micrometers or a surface layer substantially free of particles.

### Example 3

### Preparation of Control Element C-2

Control Element C-2 was a commercially available inkjet non-porous receiver paper containing an ink receiving layer comprised of a high amount of gelatin, "Kodak Inkjet Photo Paper", catalogue No. 1181197 from Eastman Kodak Co. The clement was printed the same as in Example 1. The surface gloss, and the ink dry time were measured the same as in Example 1. The measured surface gloss at 60 degrees was 84 and the ink dry time was measured to be 150 seconds.

### Preparation of Element 12

A coating composition (Solution S-2) was prepared the same as in Element 3. Solution S-2 was coated over the Control Element C-2 using a calibrated coating knife, and dried to remove substantially all solvent components. The thickness of this layer was measured to be about 3 ± 1 µm. The element was printed the same as in Example 1. The surface gloss, and the ink dry time were measured the same as in Example 1. The measured surface gloss at 60 degrees was 57 and the ink dry time was measured to be 20 seconds, much faster than that measured for Control Element C-2.

### Example 4

### Preparation of Control Element C-3

Control Element C-3 was a commercially available inkjet porous receiver paper containing ink receiving layer comprising a high amount of silica fine particles, "Epson Premium Glossy Photo Paper", catalogue No. SO41286 from Epson.

### Preparation of Element 13

A coating composition (Solution S-2) was prepared the same as in Element 3 and was coated over the Control Element C-3 using a calibrated coating knife, and dried to remove substantially all solvent components. The thickness of this layer was measured to be about 4 ± 2 µm.

### Preparation of Control Element C-4

A coating composition (Solution S-11) was prepared by combining fumed alumina (Cab-O-Sperse® PG003, Cabot Corp.), poly(vinyl alcohol) (Gohsenol® GH-23A, Nippon Gohsei Co., Ltd.) and 2,3-dihydroxy-1,4-dioxane (Clariant Corp.) in a weight ratio of 88:10:2 to give an aqueous coating formulation of 30 % solids by weight.

A coating solution (Solution S-12) was prepared by combining fumed alumina (Cab-O-Sperse® PG003, Cabot Corp.), poly(vinyl alcohol) (Gohsenol® GH-23A, Nippon Gohsei Co.) and a copolymer of (vinylbenzyl)trimethylammonium chloride and divinylbenzene (87:13 molar ratio) in a weight ratio of 85:3:12 to give an aqueous coating formulation of 10% solids by weight. The fumed alumina particles have a primary particle size of from about 7 to about 40 nm in diameter and are aggregated up to about 150 nm. Surfactants Zonyl® FSN (E. I. du Pont de Nemours and Co.) and Olin@ 10G (Dixie Chemical Co.) were added in small amounts as coating aids.

Both coating compositions were metered to a multiple-slot-die coating apparatus and coated simultaneously at 40°C, with Solution S-11 being located below (closer to the support than) Solution S-12, onto a base support comprised of a polyethylene-coated paper base which had been previously subjected to corona discharge treatment. The coated support immediately entered the drying section of the coating machine to remove substantially all solvent components and form a two-layer image receiving element. The thicknesses of the bottom and topmost layers were 40 µm and 2 µm, respectively.

### Preparation of Element 14

A coating composition (Solution S-2) was prepared the same as in Element 3 and was coated over the Control Element C-4 using a calibrated coating knife, and dried to remove substantially all solvent components. The thickness of this layer was measured to be about 4 ± 2 µm.

### Preparation of Control Element C-5

A coating composition for a base layer was prepared by mixing 254 dry g of precipitated calcium carbonate Albagloss-s® (Specialty Minerals Inc.) as a 70 wt. % solution, 22 dry g of silica gel Gasil® 23F (Crosfield Ltd.), 2.6 dry g of poly(vinyl alcohol) Airvol® 125 (Air Products) as a 10 wt. % solution and 21 dry g of styrene-butadiene latex CP692NA® (Dow Chemicals) as a 50 wt. % solution. The wt. % solids of the coating composition was adjusted to 35 wt. % by adding water. The base layer coating composition was bead-coated at 25 ° C on a paper support with basis weight of 185 g/m² (Eastman Kodak Co.) and dried by forced air at 45°C. The thickness of the base layer was 25 µm.

### Preparation of Element 15

A coating composition (Solution S-2) was prepared the same as in Element 3 and was coated over the Control Element C-5 using a calibrated coating knife, and dried to remove substantially all solvent components. The thickness of this layer was measured to be about 2 ± 0.5 µm.

### Measurement of ink dry time

A drop (from a 5 microliter capillary tube) of a magenta inkjet ink, prepared using a standard formulation with Dye 6 from U.S. Patent 6,001,161, was placed on each unprinted element and the time that it took for this spot to become dry to the touch was measured as the "ink drying time".

### Printing and dye stability testing

The above elements and control elements of Example 4 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) were read using an X-Rite ® 820 densitometer. The cyan density is reported in Table 5. The printed elements were then subjected to 4 days exposure to a nitrogen flow containing 5 ppm ozone. The density of each patch was read after the exposure test using an X-Rite® 820 densitometer. The % dye retention was calculated as the ratio of the density after the exposure test to the density before the exposure test. The results for cyan D-max are reported in Table 7.

**Table 7**

| **Element** | **Particle in lower ink receiving layer** | **Particle in upper ink receiving layer** | **Cyan D-max** | **% dye retention cyan D-max** | **60° gloss** | **Ink drying time (seconds)** |
|---|---|---|---|---|---|---|
| 13 | Silica | PE-2 | 1.6 | 96.3 | 71 | 20 |
| 14 | Fumed alumina | PE-2 | 1.6 | 95.0 | 49 | 20 |
| 15 | Calcium carbonate, latex | PE-2 | 2.0 | 95.5 | 20 | 30 |
| C-3 | Silica | None | 2.1 | 19.7 | 41 | 30 |
| C-4 | Fumed alumina | None | 1.9 | 19.6 | 62 | 45 |
| C-5 | Calcium carbonate, latex | None | 0.7 | 80.3 | 6 | 20 |

The above results show that improved dye stability for the element can be achieved, while maintaining surface gloss and ink dry time, with a multilayer ink receiving layer structure, particularly when the upper layer contains porous polyester particles that have a mean diameter of less than 0.5 micrometers.

### Example 5

### 2-step Preparation of Bead Containing Polyester-urethane (PEU-1).

Polyester-diol prepolymer: This reaction was set up and run in an identical manner as that described in step 1 of the preparation of PEC-1 described below using Maleic anhydride (107.61 g, 1.10 mol), neopentyl glycol (137.15 g, 1.32 mol), and Fascat 4100(~ 5 mg, catalytic). The alcohol end groups were determined by direct quantification using 1H NMR with an internal standard. The determined value of 2.0 meq ROH/g polymer corresponds to a number average molecular weight of 1036.3 g/mol.

Particles containing polyester-urethane: An organic phase was prepared consisting of the polycster-diol oligomer from the previous step (10.00 g) toluene (55.20 g), Desmodur N3300® triisocyanate resin (3.80 g), stannous octanoate (0.05 g), dibutyltin dilaurate (0.05 g), 80% divinylbenzene (41.40g, mixture *of m* and *p* isomers with remainder being ethylstyrene), hexadecane (2.21 g), and AIBN initiator (1.03 g). The components were stirred until a clear, heterogeneous solution resulted. An aqueous phase was prepared consisting of sodium dodecylsulfate (4.40 g) dissolved in deionized water (120.00). The two phases were combined and emulsified using a Silverson L4R mixer at the highest speed for 10 minutes followed by passage twice through an M-110T Microfluidizer® (sold by Microfluidics). The resulting emulsion was poured into a 3-neck 2000 ml round bottom flask outfitted with a mechanical stirrer, condenser, and nitrogen inlet and was bubble degassed with nitrogen for 10 minutes. The emulsion was heated for 16 hours with vigorous stirring in a thermostatted water bath at 70°C and the toluene was removed via rotary evaporation. The resulting particle dispersion had 10.23% solids. Analysis of the product dispersion using a Horiba® LA-920 particle sizing instrument showed a single mode with a mean particle diameter of 0.153 microns.

### Preparation of Element 16

A coating composition was prepared from 48.7 wt. % of aqueous dispersion of PEU-1 (10.23 wt % solids in water), 5.0 wt. % poly(vinyl alcohol), PVA, (Gohsenol® GH-17 from Nippon Gohsei Co.), and 46.3 wt. % water. [The relative proportions of porous organic particle to PVA are therefore 50/50 by weight]. The coating composition was coated over the Control Element C-5 using a calibrated coating knife, and dried to remove substantially all solvent components.

### Example 6

### 3-step Preparation of Porous Beads Containing Polyester-carbonate (PEC-1)

Polyester-diol prepolymer: Fumaric acid (100.00 g, 6.61x10⁻¹ mol), cyclohexanedimethanol (174.04 g, 1.20 mol), and Fascat 4100 (~ 10 mg, catalytic) were combined in a 500 ml single neck round bottom flask outfitted with a mechanical stirrer and a side arm leading to a condenser assembly with a graduated cylinder to measure the volume of condensate. The reaction was placed in a bath filled with a low melting heating alloy and the temperature was ramped from 150°C to 220°C over 50 minutes then held at 220°C for 200 minutes at which point ~32 ml of condensate had been collected. The molten polyester was cooled to room temperature, frozen in liquid nitrogen, broken up with a hammer and dried in a vacuum oven overnight at 60°C. The alcohol end groups were determined by dissolving the polyester in deuterochloroform, endcapping the polyester with trifluoroacetylimidazole, integrating the ¹⁹F NMR end group peaks, and normalizing to an internal standard. The determined value of 2.28 meq ROH/g polymer corresponds to a number average molecular weight of 877.19 g/mol.

Unsaturated polyester-carbonate: The unsaturated polyester diol oligomer from the previous step (43.85 g, 0.05 mol) and trimethylamine (22.26 g, 0.22 mol) were dissolved in dichloromethane (150 g). While stirring at room temperature, a solution of bisphenol A bis(chloroformate) (47.66 g, 0.05 g) in dichloromethane (50 ml) was slowly added over ~20 min. The reaction was allowed to proceed at room temperature for two hours, by which time it had become notably viscous and was further diluted 100 g dichloromethane. The product solution was then extracted once with 250 ml of 2% hydrochloric acid, and twice with water. The product solution was precipitated into methanol and dried overnight in a vacuum oven at 60°C. Analysis by Differential scanning calorimetry showed a Tg of 89.4°C. Size exclusion chromatography in hexafluoroisopropanol showed Mn = 1,390 and Mw = 80,700. The broad curve suggested that the polymer may be highly branched.

Particles containing polyester-co-carbonate: An organic phase was prepared consisting of the unsaturated polyester-co-carbonate from the previous step (10.00 g) toluene (20.00 g), chloromethylstyrene (5.00 g), 80% divinylbenzene (5.00g, mixture *of m* and *p* isomers with remainder being ethylstyrene), hexadecane (0.80 g), and Vazo 52® initiator (0.20 g). The components were stirred until a clear, heterogeneous solution resulted. An aqueous phase was prepared consisting of dodecanethiol-endcapped polyacrylamide decamer surfactant (1.60 g, prepared as described in US 6,127,453 column 9 lines 40-55) dissolved in deionized water (120.00). The two phases were combined and sonicated using a Vibra Cell ® probe sonicator (Sonics & Materials Inc.) at the highest power setting for 10 minutes, then transferred to a 500 ml 3-neck round bottomed flask outfitted with a condenser, nitrogen inlet, and mechanical stirrer. The reaction mixture was bubble degassed with nitrogen for 10 minutes and heated for 16 hours with vigorous stirring at 60°C in a thermostatted water bath. The toluene was then removed via rotary evaporation and dimethylethanolamine (1.17 g) was added. The quaternization reaction was allowed to proceed at 60°C for 16 hours and the excess amine and surfactant was removed via dialysis using 12-14K cutoff cellulose dialysis tubing for 16 hours to yield a product dispersion of 13.3% solids. Analysis of the product dispersion using a Horiba® LA-920 particle sizing instrument showed a bimodal distribution with a mean particle diameter of 1.462 microns, a major mode at 0.36 microns, and a smaller mode, presumably due to secondary aggregation, at ~6 microns. Preparation of Element 17

A coating composition was prepared from 38.0 wt. % of aqueous dispersion PEC-1 (13.33 wt % solids in water), 5.0 wt. % poly(vinyl alcohol), PVA, (Gohsenol® GH-17 from Nippon Gohsei Co.), and 57.0 wt. % water. [The relative proportions of porous polyester particle to PVA are therefore 50/50 by weight]. The coating composition was coated over the Control Element C-5 using a calibrated coating knife, and dried to remove substantially all solvent components. The thickness of the dry ink receiving layer was measured to be about 9 ± 2 µm.

The above elements of Example 5 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) were measured to be 1.4 for element 16 and 1.3 for element 17, much higher than the density measured for control element C-5.

## Claims

1. An ink recording element comprising a support and at least two ink receiving layers, wherein at least one of said at least two ink receiving layers comprises porous organic particles and is porous, wherein said porous organic particles comprise unsaturated condensation polymer reacted with a vinyl monomer, and wherein said porous organic particles comprise at least 80 weight % of an individual layer.

2. The ink recording element of claim 1 wherein said porous organic particles comprise at least one layer below the topmost layer of said ink recording element, wherein said at least one layer comprising said porous organic particles below said topmost layer of said ink recording element is porous.

3. The ink recording element of claim 1 wherein said porous organic particles comprise the topmost layer of said ink recording element, wherein said topmost layer of said ink recording element comprising organic particles is porous.

4. The ink recording element of claim 3 comprising at least one layer below the topmost layer of said ink recording element, wherein said at least one layer below said topmost layer comprises inorganic particles, wherein said at least one layer below said topmost layer is free of said organic particles, and wherein said at least one layer below said topmost layer of said ink recording element is porous.

5. The ink recording element of claim 1 wherein said unsaturated condensation polymer comprises ionic groups having quaternary ammonium moieties.

6. The ink recording element of claims 1-5 wherein said porous organic particles comprise porous polyester particles.

7. The ink recording element of claim 6 wherein said porous polyester particles comprise particles having a mean diameter of less than 0.5 micrometers.

8. The ink recording element of claim 2 wherein said porous organic particles comprise porous polyester particles, wherein said porous polyester particles are also present in the topmost layer of said ink recording element and wherein said porous polyester particles in said at least one layer below said topmost layer comprise particles having a size greater than 0.5 micrometers.

9. The ink recording element of claim 6 wherein said porous polyester particles comprise precursor polyester comprising at least one member the group consisting of maleic, fumaric, itaconic, phenylenediacrylic, citraconic and mesaconic acid.

## Patentansprüche

1. Tintenstrahlaufzeichnungselement mit einem Träger und mindestens zwei Tintenempfangsschichten, worin mindestens eine der mindestens zwei Tintenempfangsschichten poröse organische Partikel umfasst und porös ist, worin die porösen organischen Partikel ungesättigtes Kondensationspolymer enthalten, reagiert mit einem Vinylmonomer, und worin die porösen organischen Partikel mindestens 80 Gew.-% einer einzelnen Schicht umfassen.

2. Tintenstrahlaufzeichnungselement nach Anspruch 1, worin die porösen organischen Partikel mindestens eine Schicht unterhalb der obersten Schicht des Tintenstrahlaufzeichnungselements umfassen, worin die mindestens eine Schicht, die die porösen organischen Partikel unterhalb der obersten Schicht des Tintenstrahlaufzeichnungselements enthält, porös ist.

3. Tintenstrahlaufzeichnungselement nach Anspruch 1, worin die porösen organischen Partikel die oberste Schicht des Tintenstrahlaufzeichnungselements umfassen, und worin die oberste Schicht des Tintenstrahlaufzeichnungselements, welche organische Partikel enthält, porös ist.

4. Tintenstrahlaufzeichnungselement nach Anspruch 3 mit mindestens einer Schicht unterhalb der obersten Schicht des Tintenstrahlaufzeichnungselements, worin die mindestens eine Schicht unterhalb der obersten Schicht anorganische Partikel umfasst, worin die mindestens eine Schicht unterhalb der obersten Schicht frei von den organischen Partikeln ist, und worin die mindestens eine Schicht unterhalb der obersten Schicht des Tintenstrahlaufzeichnungselements porös ist.

5. Tintenstrahlaufzeichnungselement nach Anspruch 1, worin das ungesättigte Kondensationspolymer ionische Gruppen mit quaternären Ammoniumresten enthält.

6. Tintenstrahlaufzeichnungselement nach Anspruch 1-5, worin die porösen organischen Partikel poröse Polyesterpartikel enthalten.

7. Tintenstrahlaufzeichnungselement nach Anspruch 6, worin die porösen Polyesterpartikel Partikel mit einem mittleren Durchmesser von kleiner als 0,5 µm enthalten.

8. Tintenstrahlaufzeichnungselement nach Anspruch 2, worin die porösen organischen Partikel poröse Polyesterpartikel enthalten, worin die porösen Polyesterpartikel auch in der obersten Schicht des Tintenstrahlaufzeichnungselements vorhanden sind und worin die porösen Polyesterpartikel in der mindestens einen Schicht unterhalb der obersten Schicht Partikel mit einer Größe von größer als 0,5 µm enthalten.

9. Tintenstrahlaufzeichnungselement nach Anspruch 6, worin die porösen Polyesterpartikel Vorläuferpolyester umfassen mit mindestens einem Mitglied der Gruppe, die aus Malein-, Fumar-, Itakon-, Phenylendiacryl-, Citracon- und Mesaconsäure besteht.

## Revendications

1. Elément pour l'enregistrement par jet d'encre comprenant un support et au moins deux couches réceptrices d'encre, dans lequel au moins l'une desdites au moins deux couches réceptrices d'encre comprend des particules organiques poreuses et est poreuse, où lesdites particules organiques poreuses comprennent un polymère de condensation insaturé ayant réagi avec un monomère vinylique, et dans lequel lesdites particules organiques poreuses représentent au moins 80% en poids d'une couche individuelle.

2. Elément pour l'enregistrement par jet d'encre selon la revendication 1, dans lequel lesdites particules organiques poreuses constituent au moins une couche sous la couche supérieure dudit élément pour l'enregistrement par jet d'encre, dans lequel ladite au moins une couche comprenant lesdites particules organiques poreuses sous ladite couche supérieure dudit élément pour l'enregistrement par jet d'encre est poreuse.

3. Elément pour l'enregistrement par jet d'encre selon la revendication 1, dans lequel lesdites particules organiques poreuses constituent la couche supérieure dudit élément pour l'enregistrement par jet d'encre, où ladite couche supérieure dudit élément pour l'enregistrement par jet d'encre comprenant des particules organiques est poreuse.

4. Elément pour l'enregistrement par jet d'encre selon la revendication 3 comprenant au moins une couche sous la couche supérieure dudit élément pour l'enregistrement par jet d'encre, dans lequel ladite au moins une couche sous ladite couche supérieure comprend des particules inorganiques, où ladite au moins une couche sous ladite couche supérieure est exempte desdites particules organiques et où ladite au moins une couche sous ladite couche supérieure dudit élément pour l'enregistrement par jet d'encre est poreuse.

5. Elément pour l'enregistrement par jet d'encre selon la revendication 1, dans lequel ledit polymère de condensation insaturé comprend des groupes ioniques ayant des radicaux ammonium quaternaire.

6. Elément pour l'enregistrement par jet d'encre selon les revendications 1 à 5, dans lequel lesdites particules organiques poreuses comprennent des particules poreuses de polyester.

7. Elément pour l'enregistrement par jet d'encre selon la revendication 6, dans lequel lesdites particules poreuses de polyester comprennent des particules d'un diamètre moyen inférieur à 0,5 micromètres.

8. Elément pour l'enregistrement par jet d'encre selon la revendication 2, dans lequel lesdites particules organiques poreuses comprennent des particules poreuses de polyester, où lesdites particules poreuses de polyester sont également présentes dans la couche supérieure dudit élément pour l'enregistrement par jet d'encre et où lesdites particules poreuses de polyester dans ladite au moins une couche sous ladite couche supérieure comprennent des particules ayant une taille supérieure à 0,5 micromètres.

9. Elément pour l'enregistrement par jet d'encre selon la revendication 6, dans lequel lesdites particules poreuses de polyester comprennent un précurseur polyester comprenant au moins un membre parmi le groupe comprenant l'acide maléique, fumarique, itaconique, phénylènediacrylique, citraconique et mésaconique.
